



US009389523B2

(12) **United States Patent**  
Nakata et al.

(10) **Patent No.:** US 9,389,523 B2  
(45) **Date of Patent:** Jul. 12, 2016

(54) **ELECTROPHOTOGRAPHIC PHOTOSENSITIVE MEMBER, AND ELECTROPHOTOGRAPHIC APPARATUS AND PROCESS CARTRIDGE EACH INCLUDING THE ELECTROPHOTOGRAPHIC PHOTOSENSITIVE MEMBER**

(71) **Applicant:** CANON KABUSHIKI KAISHA, Tokyo (JP)

(72) **Inventors:** Koichi Nakata, Kashiwa (JP); Shinji Takagi, Yokohama (JP); Nobuo Kosaka, Gotemba (JP); Koichi Suzuki, Yokohama (JP)

(73) **Assignee:** CANON KABUSHIKI KAISHA, Tokyo (JP)

(\*) **Notice:** Subject to any disclaimer, the term of this patent is extended or adjusted under 35 U.S.C. 154(b) by 0 days.

(21) **Appl. No.:** 14/191,414

(22) **Filed:** Feb. 26, 2014

(65) **Prior Publication Data**

US 2014/0255837 A1 Sep. 11, 2014

(30) **Foreign Application Priority Data**

Mar. 7, 2013 (JP) ..... 2013-045715  
Feb. 24, 2014 (JP) ..... 2014-032962

(51) **Int. Cl.**

G03G 5/06 (2006.01)  
G03G 21/18 (2006.01)  
G03G 5/147 (2006.01)

(52) **U.S. Cl.**

CPC ..... G03G 5/0607 (2013.01); G03G 5/0605 (2013.01); G03G 5/0609 (2013.01); G03G 5/0629 (2013.01); G03G 5/14708 (2013.01); G03G 21/1803 (2013.01)

(58) **Field of Classification Search**  
CPC ..... G03G 5/0517; G03G 7/0026  
See application file for complete search history.

(56) **References Cited**

U.S. PATENT DOCUMENTS

5,665,500 A 9/1997 Suzuki  
7,364,824 B2 4/2008 Kikuchi et al.  
(Continued)

FOREIGN PATENT DOCUMENTS

EP 1 182 183 A1 2/2002  
EP 2 469 341 A1 6/2012

(Continued)

OTHER PUBLICATIONS

Nakata, et al., U.S. Appl. No. 14/191,413, filed Feb. 26, 2014.  
European Search Report dated Oct. 27, 2014 in European Application No. 14000812.9.

*Primary Examiner* — Hoa V Le

(74) **Attorney, Agent, or Firm:** Fitzpatrick, Cella, Harper and Scinto

(57) **ABSTRACT**

Provided is an electrophotographic photosensitive member excellent in suppression of image deletion and electric potential variation. The surface layer of the electrophotographic photosensitive member comprises a hole transporting substance. The hole transporting substance is one of a compound consisting of a carbon atom and a hydrogen atom, or a compound consisting of a carbon atom, a hydrogen atom, and an oxygen atom. The hole transporting substance comprises a conjugate structure containing 24 or more  $sp^2$  carbon atoms. The conjugate structure comprises a condensed polycyclic structure comprising 12 or more  $sp^2$  carbon atoms. A ratio of a number of  $sp^2$  carbon atoms is 55% or more based on a total number of carbon atoms in the hole transporting substance, and a ratio of a number of  $sp^3$  carbon atoms is 10% or more based on a total number of carbon atoms in the hole transporting substance.

8 Claims, 2 Drawing Sheets



(56)

**References Cited**

U.S. PATENT DOCUMENTS

8,354,210 B2 1/2013 Takaki et al.  
8,632,931 B2 1/2014 Sekido et al.  
2006/0183042 A1 \* 8/2006 Huang ..... C07C 13/567  
430/58.05  
2008/0138725 A1 \* 6/2008 Fujiwara ..... G03G 5/0525  
430/48

2009/0278446 A1 11/2009 Igawa et al.  
2011/0180791 A1 7/2011 Pan et al.

FOREIGN PATENT DOCUMENTS

JP 8-272126 A 10/1996  
JP 2001-242656 A 9/2001  
JP 2007-279446 A 10/2007  
JP 2012-502304 A 1/2012

\* cited by examiner

*FIG. 1**FIG. 2**FIG. 3*

FIG. 4



FIG. 5



## 1

**ELECTROPHOTOGRAPHIC  
PHOTOSENSITIVE MEMBER, AND  
ELECTROPHOTOGRAPHIC APPARATUS  
AND PROCESS CARTRIDGE EACH  
INCLUDING THE  
ELECTROPHOTOGRAPHIC  
PHOTOSENSITIVE MEMBER**

## BACKGROUND OF THE INVENTION

## 1. Field of the Invention

The present invention relates to an electrophotographic photosensitive member, and an electrophotographic apparatus and a process cartridge each including the electrophotographic photosensitive member.

## 2. Description of the Related Art

Technologies for improving the material, physical properties, and the like of the surface of the electrophotographic photosensitive member (photosensitive member) containing an organic photoconductive substance have been investigated in order that the durability of the electrophotographic photosensitive member may be improved.

However, the improvement of the durability of the electrophotographic photosensitive member tends to be liable to cause image deletion or electric potential variation.

The image deletion is considered to be caused by: the deterioration of a material in the surface layer of the electrophotographic photosensitive member due to, for example, ozone or a nitrogen oxide produced by charging of the electrophotographic photosensitive member; or the reduction in surface resistance of the surface layer due to the adsorption of moisture to the surface of the electrophotographic photosensitive member. The image deletion is liable to remarkably occur particularly under a high-temperature and high-humidity environment.

Similarly, the electric potential variation is liable to occur owing to the deterioration of a constituent material caused by repeated use of the electrophotographic photosensitive member.

Japanese Patent Application Laid-Open No. H08-272126 and Japanese Patent Application Laid-Open No. 2001-242656 each describe that the gas permeability and ozone resistance of the electrophotographic photosensitive member are improved, and the image density variation thereof is alleviated, by incorporating a specific additive into the electrophotographic photosensitive member.

Japanese Patent Application Laid-Open No. 2007-279446 describes that the incorporation of a specific additive into a photosensitive layer can improve the stability of electrical characteristics and hence suppresses the occurrence of an image failure such as a memory.

In recent years, an improvement in durability of an electrophotographic apparatus has been progressed, and hence a demand for additional alleviation of the image deletion and the electric potential variation has been growing.

## SUMMARY OF THE INVENTION

In view of the foregoing, the present invention is directed to providing an electrophotographic photosensitive member excellent in suppression of image deletion and electric potential variation. Further, the present invention is directed to providing an electrophotographic apparatus and a process cartridge each including the electrophotographic photosensitive member.

According to one aspect of the present invention, there is provided an electrophotographic photosensitive member

## 2

comprising: a support; and a photosensitive layer formed on the support, wherein a surface layer of the electrophotographic photosensitive member comprises a hole transporting substance, wherein, the hole transporting substance is one of: 5 a compound consisting of a carbon atom and a hydrogen atom; and a compound consisting of a carbon atom, a hydrogen atom and an oxygen atom, the hole transporting substance comprises a conjugate structure comprising 24 or more  $sp^2$  carbon atoms, wherein, the conjugate structure comprises a condensed polycyclic structure comprising 12 or more  $sp^2$  carbon atoms, a ratio of a number of  $sp^2$  carbon atoms is 55% or more based on a total number of carbon atoms in the hole transporting substance, and a ratio of a number of  $sp^3$  carbon atoms is 10% or more based on a total number of carbon atoms in the hole transporting substance.

According to another aspect of the present invention, there is provided a process cartridge detachably mountable to a main body of an electrophotographic apparatus, wherein the process cartridge integrally supports: the above-described electrophotographic photosensitive member; and at least one device selected from the group consisting of a charging device, a developing device, and a cleaning device.

According to further aspect of the present invention, there is provided an electrophotographic apparatus comprising: the above-described electrophotographic photosensitive member; a charging device; an exposing device; a developing device; and a transferring device.

According to the present invention, there is provided the electrophotographic photosensitive member excellent in suppression of image deletion and electric potential variation. Further, according to the present invention, provided are the electrophotographic apparatus and the process cartridge each including the above-described electrophotographic photosensitive member.

Further features of the present invention will become apparent from the following description of exemplary embodiments with reference to the attached drawings.

## BRIEF DESCRIPTION OF THE DRAWINGS

FIG. 1 is a view illustrating an example of a layer construction of an electrophotographic photosensitive member.

FIG. 2 is a view illustrating an example of a layer construction of an electrophotographic photosensitive member.

FIG. 3 is a view illustrating an example of a layer construction of an electrophotographic photosensitive member.

FIG. 4 is a view illustrating an example of a schematic construction of an electrophotographic apparatus including a process cartridge having an electrophotographic photosensitive member.

FIG. 5 is a view illustrating an example of a schematic construction of a process cartridge including an electrophotographic photosensitive member according to the present invention.

## DESCRIPTION OF THE EMBODIMENTS

A surface layer of an electrophotographic photosensitive member of the present invention includes a hole transporting substance, and the hole transporting substance is a compound consisting of a carbon atom and a hydrogen atom, or consisting of a carbon atom, a hydrogen atom, and an oxygen atom. Further, the hole transporting substance includes a conjugate structure containing 24 or more  $sp^2$  carbon atoms and the conjugate structure includes a condensed polycyclic structure containing 12 or more  $sp^2$  carbon atoms. In addition to those characteristics, the electrophotographic photosensitive mem-

ber of the present invention is characterized in that the ratio of the number of the  $sp^2$  carbon atoms to the total number of carbon atoms in the hole transporting substance is 55% or more, and the ratio of the number of the  $sp^3$  carbon atoms to the total number of carbon atoms in the hole transporting substance is 10% or more.

The inventors of the present invention have considered that one cause for image deletion is that an aromatic amine compound that has heretofore been used as a hole transporting substance is excellent in hole injecting performance and hole transporting performance, but tends to be susceptible to deterioration such as oxidation. The surface of the electrophotographic photosensitive member is considered to be susceptible to deterioration such as oxidation particularly due to ozone or a nitrogen oxide produced in a process for the charging of the surface of the electrophotographic photosensitive member.

The inventors of the present invention have considered that one cause for the image deletion is that the amine structure of the hole transporting substance to be incorporated into the surface layer of an ordinary electrophotographic photosensitive member causes a chemical change. In view of the foregoing, the inventors of the present invention have searched for a hole transporting substance for the electrophotographic photosensitive member independent of an amine structure, and have reached the present invention.

Specifically, the substance is a compound (hole transporting substance) consisting of a carbon atom and a hydrogen atom, or consisting of a carbon atom, a hydrogen atom, and an oxygen atom, and is a compound having a good hole transporting performance even when used in the electrophotographic photosensitive member.

The molecular structure of the hole transporting substance needs to be such a structure that a conjugated double bond system has a certain spread in the molecule and an electron is delocalized. Further, the substance may need to have a large number of condensed polycyclic structures (condensed polycyclic aromatic structures) each having specific planarity in order that the giving and receiving of holes may be efficiently performed and the stability of a cation in a transition state may be improved.

Japanese Patent Translation Publication No. 2012-502304 describes an example in which a polymer of an aromatic hydrocarbon compound is used as a hole transporting substance. However, when the polymer is used as it is in the surface layer, the durability of the electrophotographic photosensitive member is not sufficient and hence a binder resin may need to be used in combination. In view of the foregoing, the ratio of the  $sp^3$  carbon atom such as an alkyl group needs to be increased in order that the compatibility of the polymer with the binder resin may be improved. On the other hand, however, the following demerit arises: the  $sp^3$  carbon atom is not involved in a conjugate system and reduces a hole transporting performance. Accordingly, it cannot be said that the control of both the ratio and the hole transporting performance has been sufficient.

The hole transporting substance of the present invention needs to be such that the ratio of the number of  $sp^2$  carbon atoms in the hole transporting substance falls within a certain range in order that a high hole transporting performance may be secured. In addition, the presence of the  $sp^3$  carbon atom at a moderate abundance ratio in the molecule contributes to the improvement of the hole transporting performance, the increase in hole mobility, and the adjustment of the energy level of the hole transporting substance. On the other hand, as described above, the ratio of the number of the  $sp^3$  carbon atoms needs to be controlled to the ratio of the number

described above because a hole transporting performance is inhibited when the ratio is excessively large.

That is, the hole transporting substance of the present invention is a compound having the following features.

5 The hole transporting substance has a molecular structure having a conjugate structure containing 24 or more  $sp^2$  carbon atoms. The term "conjugate structure" refers to such a structure that the  $sp^2$  carbon atoms are continuously bonded, and the conjugated double bonds in each of which a double bond 10 and a single bond are alternately present are continuously present. The conjugate structure means a structure that enables the delocalization of an electron in the molecule.

The conjugate structure is more preferably a conjugate structure containing a structure in which 28 or more  $sp^2$  15 carbon atoms are continuously linked. The structure is still more preferably a conjugate structure containing 36 or more  $sp^2$  carbon atoms.

The number of the  $sp^2$  carbon atoms of the hole transporting substance is preferably 120 or less, more preferably 60 or 20 less from the viewpoints of, for example, a film forming ability, its compatibility with a material for forming the surface layer, and film strength.

In addition, at the same time, the hole transporting substance of the present invention has, in the conjugate structure, 25 a condensed polycyclic structure containing 12 or more  $sp^2$  carbon atoms. The term "condensed polycyclic structure" means a structure in which two or more cyclic structures like benzene rings are adjacent to each other.

The hole transporting substance of the present invention 30 preferably has two condensed polycyclic structures and more preferably has three or more condensed polycyclic structures. The number of the  $sp^2$  carbon atoms in each condensed polycyclic structure is preferably 14 or more, more preferably 16 or more from the viewpoint of the hole transporting performance. When the hole transporting substance has two or more condensed polycyclic structures, at least one condensed polycyclic structure preferably contains 16 or more  $sp^2$  carbon atoms.

The number of the  $sp^2$  carbon atoms forming each condensed polycyclic structure is preferably 20 or less, more preferably 18 or less from the viewpoints of the film forming ability and the compatibility with the material for forming the surface layer.

With regard to a ring structure forming each condensed 45 polycyclic structure, it is suitable that a conjugate structure spreads in a planar manner. Therefore, the condensed polycyclic structure is preferably formed of a five-membered ring or a six-membered ring in order that a planar structure may be formed. The number of the ring structures forming the condensed polycyclic structure, which is 2 or more, is preferably 50 3 or more in order that the hole transporting performance may be made additionally suitable.

With regard to the ring structures forming each condensed 55 polycyclic structure, the condensed polycyclic structure is preferably formed of 6 or less rings and is more preferably formed of 5 or less rings from the viewpoints of film formability and the flexibility of the molecule. That is, a condensed polycyclic structure formed of 3 or 4 rings is most preferred.

The hole transporting substance of the present invention 60 has at least one unit (one) of the condensed polycyclic structure as a partial structure. The hole transporting substance preferably has two or more units of the condensed polycyclic structures and more preferably has three or more units of the condensed polycyclic structures from the viewpoint of additionally expressing the hole transporting performance. In addition, the number of the units of the condensed polycyclic structures in one molecule of the hole transporting substance

is preferably 10 or less, more preferably 4 or less. Those condensed polycyclic structures preferably have a structure in which the condensed polycyclic structures are bonded to each other through a single bond (the condensed polycyclic structures are directly bonded to each other).

The ratio of the number of the  $sp^2$  carbon atoms to the total number of carbon atoms in the hole transporting substance of the present invention is 55% or more in order that the hole transporting substance may express good hole transporting performance.

When the ratio of the  $sp^2$  carbon atoms becomes smaller than 55%, sufficient hole transportability is not obtained owing to the inhibitory action of an  $sp^3$  carbon atom, which is not directly involved in the hole transporting performance, on hole transport. The ratio of the number of the  $sp^2$  carbon atoms to the total number of carbon atoms is preferably 55% or more and 90% or less, and the ratio of the number of the  $sp^2$  carbon atoms is more preferably 65% or more and 85% or less.

Most of the carbon atoms of the hole transporting substance of the present invention are formed of the  $sp^3$  carbon atom and the  $sp^2$  carbon atom. The hole transporting substance of the present invention is such that the ratio of the number of the  $sp^3$  carbon atoms to the total number of carbon atoms in the hole transporting substance is 10% or more, preferably 10% or more and 45% or less, more preferably 12% or more.

When the ratio of the number of the  $sp^3$  carbon atoms falls within the range, the hole mobility increases and the energy level of the entire molecule of the hole transporting substance is moderately adjusted by moderate electron donating property of an alkyl substituent, whereby the hole transporting performance improves. In addition, the ratio contributes to the suppression of excessive stacking property between the molecules of the hole transporting substance, an improvement in dispersibility of the hole transporting substance in the layer at the time of film formation, and uniform presence of the hole transporting substance in the layer, whereby the hole transportability is improved.

The ratio is more preferably 15% or more and 35% or less, still more preferably 15% or more and 30% or less from the viewpoint of the hole transporting performance.

The hole transporting substance of the present invention is preferably a compound represented by the following formula (1).



(1)

In the formula (1),  $R^1$  and  $R^2$  each independently represent a hydrogen atom, a substituted or unsubstituted alkyl group, a substituted or unsubstituted aralkyl group, or a substituted or unsubstituted alkoxy group,  $R^3$  to  $R^6$  each independently represent a hydrogen atom, a substituted or unsubstituted alkyl group, a substituted or unsubstituted aralkyl group, a substituted or unsubstituted alkoxy group, or a substituted or unsubstituted aryl group,  $R^7$  represents a group derived from a substituted or unsubstituted arene by loss of 6 hydrogen atoms, and  $n$  represents an integer of from 1 to 10, and when  $n$  represents from 2 to 10, partial structures each represented by the following formula (2) in the formula (1) may be identical to or different from each other.



(2)

The hole transporting substance of the present invention represented by the formula (1) is described below.

Examples of the alkyl group include a methyl group, an ethyl group, an n-propyl group, an isopropyl group, an n-butyl group, an isobutyl group, a sec-butyl group, a tert-butyl group, an n-pentyl group, an isopentyl group, a neopentyl group, a tert-pentyl group, a cyclopentyl group, an n-hexyl group, a 1-methylpentyl group, a 4-methyl-2-pentyl group, a 3,3-dimethylbutyl group, a 2-ethylbutyl group, a cyclohexyl group, a 1-methylhexyl group, a cyclohexylmethyl group, a 4-tert-butylcyclohexyl group, an n-heptyl group, a cycloheptyl group, an n-octyl group, a cyclooctyl group, a tert-octyl group, a 1-methylheptyl group, a 2-ethylhexyl group, a 2-propylpentyl group, an n-nonyl group, a 2,2-dimethylheptyl group, a 2,6-dimethyl-4-heptyl group, a 3,5,5-trimethylhexyl group, an n-decyl group, an n-undecyl group, a 1-methyldecyl group, an n-dodecyl group, an n-tridecyl group, a 1-hexylheptyl group, an n-tetradecyl group, an n-pentadecyl group, an n-hexadecyl group, an n-heptadecyl group, an n-octadecyl group, and an n-eicosyl group.

Examples of the aralkyl group include a benzyl group, a phenethyl group, an  $\alpha$ -methylbenzyl group, an  $\alpha, \alpha$ -dimethylbenzyl group, a 1-naphthylmethyl group, a 2-naphthylmethyl group, an anthracenylmethyl group, a phenanthrenylmethyl group, a pyrenylmethyl group, a furfuryl group, a 2-methylbenzyl group, a 3-methylbenzyl group, a 4-methylbenzyl group, a 4-ethylbenzyl group, a 4-isopropylbenzyl group, a 4-tert-butylbenzyl group, a 4-n-hexylbenzyl group, a 4-n-nonylbenzyl group, a 3,4-dimethylbenzyl group, a 3-methoxybenzyl group, a 4-methoxybenzyl group, a 4-ethoxybenzyl group, a 4-n-butoxybenzyl group, a 4-n-hexyloxybenzyl group, and a 4-n-nonyloxybenzyl group.

Examples of the alkoxy group include a methoxy group, an ethoxy group, an n-propoxy group, an isopropoxy group, an n-butoxy group, an isobutoxy group, a sec-butoxy group, an n-pentyloxy group, a neopentyloxy group, a cyclopentyloxy group, an n-hexyloxy group, a 3,3-dimethylbutyloxy group, a 2-ethylbutyloxy group, a cyclohexyloxy group, an n-heptyloxy group, an n-octyloxy group, a 2-ethylhexyloxy group, an n-nonyloxy group, an n-decyloxy group, an n-undecyloxy group, an n-dodecyloxy group, an n-tridecyloxy group, an n-tetradecyloxy group, an n-pentadecyloxy group, an n-hexadecyloxy group, an n-heptadecyloxy group, an n-octadecyloxy group, and an n-eicosyloxy group.

Examples of the aryl group include: a phenyl group, a biphenyl group, a naphthyl group, a fluorenyl group, an anthracenyl group, a phenanthrenyl group, a fluoranthenyl group, a pyrenyl group, a triphenylenyl group; a monovalent group derived from tetracene; a monovalent group derived from chrysene; a monovalent group derived from pentacene; a monovalent group derived from acenaphthene; an acenaphthylene group; a monovalent group derived from perylene; a monovalent group derived from coronulene; and a monovalent group derived from coronene. Further, the aryl group may be a compound with structure in which those condensed polycyclic structures each having a conjugate structure are linked to each other directly or through a conjugated double bond group.

$R^7$  represents a group obtained by removing 6 hydrogen atoms from a substituted or unsubstituted arene. An arene

with structure in which multiple rings typified by a benzene structure further linked can be applied as the structure of the arene in R<sup>7</sup>. Of such arene structures, a condensed polycyclic structure having a conjugate structure and having a planar structure is suitable as described above. The following structure is preferred as the arene structure: a naphthalene structure, a fluorene structure, an anthracene structure, a phenanthrene structure, a fluoranthene structure, a pyrene structure, a triphenylene structure, a tetracene structure, a chrysene structure, a pentacene structure, an acenaphthene structure, an acenaphthylene structure, a perylene structure, a corannulene structure, a coronene structure, or the like. Further, the arene structure may be a structure in which those arenes are linked to each other directly or through a conjugated double bond group. Of those, the following structure is particularly suitable: a fluorene structure, an anthracene structure, a phenanthrene structure, a fluoranthene structure, or a pyrene structure.

At least one of R<sup>3</sup> to R<sup>7</sup> represents a condensed polycyclic structure, and it is preferred that two or more thereof each represent a condensed polycyclic structure.

As a substituent that any one of R<sup>1</sup> to R<sup>7</sup> may have, for example, the following groups may be given: alkyl groups such as a methyl group, an ethyl group, an n-propyl group, an n-butyl group, an isobutyl group, a tert-butyl group, an n-pentyl group, an isopentyl group, an n-hexyl group, a 1-methylpentyl group, a 3,3-dimethylbutyl group, a cyclohexyl group, an n-heptyl group, a 1-methylhexyl group, and a cyclohexylmethyl group; aralkyl groups such as a benzyl group, a phenethyl group, a naphthylmethyl group, an anthracenylmethyl group, a phenanthrenylmethyl group, a pyrenylmethyl group, and a furfuryl group; alkoxy groups such as a methoxy group, an ethoxy group, a propoxy group, a butoxy group, and a pentyloxy group; hydroxyalkyl groups such as a hydroxymethyl group, a 1-hydroxyethyl group, a 2-hydroxyethyl group, a 1-hydroxypropyl group, a 2-hydroxypropyl group, a 3-hydroxypropyl group, a 1-hydroxy-1-methylethyl group, a 1-hydroxybutyl group, a 2-hydroxybutyl group, a 3-hydroxybutyl group, a 4-hydroxybutyl group, a 2-hydroxy-2,2-dimethylpropyl group, a 2-hydroxy-1,1-dimethylethyl group, a 2-hydroxy-1,2-dimethylethyl group, a 3-hydroxy-3-methylpropyl group, a 3-hydroxy-2-methylpropyl group, a 3-hydroxy-1-methylpropyl group, a 1-hydroxypentyl group, a 2-hydroxypentyl group, a 3-hydroxypentyl group, a 4-hydroxypentyl group, a 5-hydroxypentyl group, a 3-hydroxy-3,3-dimethylpropyl group, a 3-hydroxy-2,2-dimethylpropyl group, a 3-hydroxy-1,1-dimethylpropyl group, a 3-hydroxy-1,2-dimethylpropyl group, a 3-hydroxy-1,3-dimethylpropyl group, a 4-hydroxy-4-methylbutyl group, a 4-hydroxy-3-methylbutyl group, a 4-hydroxy-2-methylbutyl group, a 4-hydroxy-1-methylbutyl group, a 1-hydroxyhexyl group, a 2-hydroxyhexyl group, a 3-hydroxyhexyl group, a 4-hydroxyhexyl group, a 5-hydroxyhexyl group, a 6-hydroxyhexyl group, a 4-hydroxy-4,4-dimethylbutyl group, a 1-hydroxyheptyl group, a 2-hydroxyheptyl group, a 3-hydroxyheptyl group, a 4-hydroxyheptyl group, a 5-hydroxyheptyl group, a 6-hydroxyheptyl group, a 7-hydroxyheptyl group, and a 5-hydroxy-5,5-dimethylpentyl group; hydroxyalkoxy groups such as a methoxymethyl group, a methoxyethyl group, a methoxypentyl group, an ethoxymethyl group, an ethoxyethyl group, an ethoxypropyl group, an ethoxybutyl group, an ethoxypentyl group, a propoxymethyl group, a propoxyethyl group, a propoxypropyl group, a propoxybutyl group, a propoxypentyl group, a butoxymethyl group, a butoxyethyl group, a butoxypropyl group, a butoxybutyl group, and a butoxypentyl group;

ester groups (alkoxycarbonyl groups) such as a formic acid ester group, an acetic acid ester group, a propionic acid ester group, a butanoic acid ester group, an acrylic acid ester group, and a methacrylic acid ester group; and various alkyl ester groups obtained by subjecting the hydroxyalkyl groups to esterification such as: a methyl formate group, an ethyl formate group, a propyl formate group, an isopropyl formate group, a butyl formate group, a pentyl formate group, and a hexyl formate group, a methyl acetate group, an ethyl acetate group, an n-propyl acetate group, an isopropyl acetate group, an n-butyl acetate group, an isobutyl acetate group, a sec-butyl acetate group, a tert-butyl acetate group, an n-pentyl acetate group, an isopentyl acetate group, a neopentyl acetate group, a tert-pentyl acetate group, an n-hexyl acetate group, an n-heptyl acetate group, an n-octyl acetate group, a methyl propionate group, an ethyl propionate group, an n-propyl propionate group, an isopropyl propionate group, an n-butyl propionate group, an isobutyl propionate group, a sec-butyl propionate group, a tert-butyl propionate group, an n-pentyl propionate group, an isopentyl propionate group, a neopentyl propionate group, a tert-pentyl propionate group, an n-hexyl propionate group, an n-heptyl propionate group, and an n-octyl propionate group; a methyl butanoate group, an ethyl butanoate group, an n-propyl butanoate group, an isopropyl butanoate group, an n-butyl butanoate group, an isobutyl butanoate group, a sec-butyl butanoate group, a tert-butyl butanoate group, an n-pentyl butanoate group, an isopentyl butanoate group, a neopentyl butanoate group, a tert-pentyl butanoate group, an n-hexyl butanoate group, an n-heptyl butanoate group, and an n-octyl butanoate group; a methyl acrylate group, an ethyl acrylate group, an n-propyl acrylate group, an isopropyl acrylate group, an n-butyl acrylate group, an isobutyl acrylate group, a sec-butyl acrylate group, a tert-butyl acrylate group, an n-pentyl acrylate group, an isopentyl acrylate group, a neopentyl acrylate group, a tert-pentyl acrylate group, an n-hexyl acrylate group, an n-heptyl acrylate group, and an n-octyl acrylate group; and a methyl methacrylate group, an ethyl methacrylate group, an n-propyl methacrylate group, an isopropyl methacrylate group, an n-butyl methacrylate group, an isobutyl methacrylate group, a sec-butyl methacrylate group, a tert-butyl methacrylate group, an n-pentyl methacrylate group, an isopentyl methacrylate group, a neopentyl methacrylate group, a tert-pentyl methacrylate group, an n-hexyl methacrylate group, an n-heptyl methacrylate group, and an n-octyl methacrylate group. In addition, the substituent may be a substituent obtained by combining a plurality of these substituents with each other.

The molecular weight of the hole transporting substance of the present invention is preferably 300 or more, more preferably 400 or more in order to express a further satisfactory hole transporting ability.

From the viewpoints of, for example, the hole transporting ability, the film forming ability, and the compatibility, the molecular weight of the hole transporting substance is preferably 3,000 or less, more preferably 2,000 or less. That is, the molecular weight is preferably 300 or more and 3,000 or less, more preferably 400 or more and 2,000 or less.

The ratio of the number of oxygen atoms in the hole transporting substance of the present invention to the number of atoms obtained by summing the number of the oxygen atoms and the number of carbon atoms is preferably 20% or less, more preferably 10% or less from the viewpoint of the hole transporting ability.

A photosensitive layer, in particular, a hole transporting layer containing the hole transporting substance of the present invention is mainly produced by an application process.

The surface layer preferably contains a binder resin in addition to the hole transporting substance. The binder resin is preferably a resin having no hole transporting function, more preferably at least one kind of resin selected from a polycarbonate resin and a polyester resin.

The hole transporting substance of the present invention is used in the surface layer of the electrophotographic photosensitive member. The hole transporting substance of the present invention may be used in a laminated electrophotographic photosensitive member or may be used in a single-layer electrophotographic photosensitive member. In the case of the laminated photosensitive member, when a hole transporting layer is positioned on a surface side, the hole transporting substance of the present invention is used in the hole transporting layer.

When the hole transporting layer is formed by further laminating two or more layers, the hole transporting substance of the present invention is incorporated into at least a hole transporting layer positioned on the surface layer.

When the hole transporting substance of the present invention is used in the single-layer photosensitive member, the hole transporting substance can be used in its photosensitive layer together with a charge generating substance.

The content (mass ratio) of the hole transporting substance of the present invention in the surface layer is preferably 50 mass % or more and 100 mass % or less, more preferably 80 mass % or more, still more preferably 90 mass % or more with respect to all hole transporting substances from the viewpoint of the suppression of deterioration due to oxidation. A layer forming the surface layer is preferably formed of a compound containing as small an amount of a heteroatom such as an amine structure as possible.

Further, the hole transporting substance of the present invention is more preferably selected from hole transporting substances each consisting of a carbon atom and a hydrogen atom for the prevention of the deterioration of the surface of the electrophotographic photosensitive member.

With regard to the electrophotographic photosensitive member, to which the hole transporting substance of the present invention is applied, the total thickness of its electrophotographic photosensitive layer has only to fall within the range of from 5  $\mu\text{m}$  to 50  $\mu\text{m}$ . Further, the thickness of the photosensitive layer is preferably 30  $\mu\text{m}$  or less. The same thickness range applies to the single-layer photosensitive member.

In addition, the thickness of the surface layer containing the hole transporting substance of the present invention is preferably 10  $\mu\text{m}$  or less, more preferably 8  $\mu\text{m}$  or less.

When the thickness of the surface layer becomes 10  $\mu\text{m}$  or less, the electrostatic capacity of the electrophotographic photosensitive member increases, and particularly when the photosensitive member is used in a contact charging-type electrophotographic apparatus, discharge deterioration of the photosensitive member in association with charging tends to increase. The hole transporting substance of the present invention is additionally suitable for a system in which such discharge deterioration due to charging frequently occurs.

#### <Electrophotographic Photosensitive Member>

Next, the entire construction of the electrophotographic photosensitive member of the present invention is described.

FIG. 1 illustrates the outline of a preferred layer construction of the electrophotographic photosensitive member in the present invention. FIG. 1 illustrates a construction in which an undercoat layer 112, a charge generating layer 113, and a hole transporting layer 114 are formed on a support 111. In this case, the hole transporting substance of the present invention is incorporated into the hole transporting layer 114 on the

side closest to the surface. FIG. 2 illustrates a construction in which an undercoat layer 122, a charge generating layer 123, a hole transporting layer 124, and a surface layer 125 are formed on a support 121. In this case, the hole transporting substance of the present invention is incorporated into the surface layer 125. Further, in the case of this layer construction, in the hole transporting layer 124, the hole transporting substance of the present invention may be used or a general known hole transporting substance such as an aromatic amine compound may be used. FIG. 3 illustrates a construction in which an undercoat layer 132 and a single-layer photosensitive layer 133 that has both a charge generating ability and a hole transporting ability are formed on a support 131. In this case, the hole transporting substance of the present invention has only to be incorporated into at least the single-layer photosensitive layer 133.

A conductive support formed of a material having electroconductivity is preferred as the support to be used in the present invention. Examples of the material for the support include: metals and alloys such as iron, copper, gold, silver, aluminum, zinc, titanium, lead, nickel, tin, antimony, indium, chromium, an aluminum alloy, and stainless steel. In addition, there may be used a support made of a metal or support made of a resin having a coat formed by depositing aluminum, an aluminum alloy, an indium oxide-tin oxide alloy, or the like through vacuum evaporation. In addition, there may also be used a support obtained by impregnating a plastic or paper with conductive particles such as carbon black, tin oxide particles, titanium oxide particles, or silver particles, or a support containing a conductive resin. The shape of the support is, for example, a cylinder-like, belt-like, sheet-like, or plate-like shape.

The surface of the support may be subjected to a cutting treatment, a surface roughening treatment, an alumite treatment, or the like for the purpose of the suppression of an interference fringe due to the scattering of laser light.

A conductive layer may be provided between the support and the undercoat layer or charge generating layer to be described later for the purposes of the suppression of an interference fringe due to the scattering of laser light or the like and the covering of a flaw of the support.

The conductive layer can be formed by: applying a conductive-layer coating solution obtained by subjecting carbon black, a conductive pigment, a resistance regulating pigment, or the like to a dispersion treatment together with a binder resin; and drying the resultant coat. A compound that undergoes curing polymerization through heating, UV irradiation, radiation irradiation, or the like may be added to the conductive-layer coating solution. The surface of the conductive layer obtained by dispersing the conductive pigment or the resistance regulating pigment tends to be roughened.

The solvent of the conductive-layer coating solution is, for example, an ether-based solvent, an alcohol-based solvent, a ketone-based solvent, or an aromatic hydrocarbon solvent. The thickness of the conductive layer is preferably 0.1  $\mu\text{m}$  or more and 50  $\mu\text{m}$  or less, more preferably 0.5  $\mu\text{m}$  or more and 40  $\mu\text{m}$  or less, still more preferably 1  $\mu\text{m}$  or more and 30  $\mu\text{m}$  or less.

Examples of the binder resin to be used for the conductive layer include: a polymer and copolymer of a vinyl compound such as styrene, vinyl acetate, vinyl chloride, an acrylic acid ester, a methacrylic acid ester, vinylidene fluoride, or trifluoroethylene; and a polyvinyl alcohol resin, a polyvinyl acetal resin, a polycarbonate resin, a polyester resin, a polysulfone resin, a polyphenylene oxide resin, a polyurethane resin, a cellulose resin, a phenol resin, a melamine resin, a silicone resin, an epoxy resin, and an isocyanate resin.

## 11

Examples of the conductive pigment and the resistance regulating pigment include particles of a metal (alloy) such as aluminum, zinc, copper, chromium, nickel, silver, or stainless steel, and plastic particles each having the metal deposited on its surface. In addition, there may be used particles of a metal oxide such as zinc oxide, titanium oxide, tin oxide, antimony oxide, indium oxide, bismuth oxide, tin-doped indium oxide, or antimony- or tantalum-doped tin oxide. One kind of those pigments may be used alone or two or more kinds thereof may be used in combination.

The undercoat layer (intermediate layer) may be provided between the support or the conductive layer and the charge generating layer for the purposes of, for example, an improvement in adhesiveness of the charge generating layer, an improvement in property by which a hole is injected from the support, and the protection of the charge generating layer from an electrical breakdown.

The undercoat layer can be formed by: applying an undercoat-layer coating solution obtained by dissolving a binder resin in a solvent; and drying the resultant coat.

Examples of the binder resin to be used for the undercoat layer include a polyvinyl alcohol resin, poly-N-vinylimidazole, a polyethylene oxide resin, ethyl cellulose, an ethylene-acrylic acid copolymer, casein, a polyamide resin, an N-methoxymethylated 6-nylon resin, a copolymerized nylon resin, a phenol resin, a polyurethane resin, an epoxy resin, an acrylic resin, a melamine resin, and a polyester resin.

Metal oxide particles may further be incorporated into the undercoat layer. An example of the metal oxide particles is particles containing titanium oxide, zinc oxide, tin oxide, zirconium oxide, or aluminum oxide. In addition, the metal oxide particles may be metal oxide particles each having a surface treated with a surface treatment agent such as a silane coupling agent.

Examples of the solvent to be used for the undercoat-layer coating solution include organic solvents such as an alcohol-based solvent, a sulfoxide-based solvent, a ketone-based solvent, an ether-based solvent, an ester-based solvent, an aliphatic halogenated hydrocarbon-based solvent, and an aromatic compound. The thickness of the undercoat layer is preferably 0.05  $\mu\text{m}$  or more and 30  $\mu\text{m}$  or less, more preferably 1  $\mu\text{m}$  or more and 25  $\mu\text{m}$  or less. Organic resin fine particles or a leveling agent may further be incorporated into the undercoat layer.

Next, the charge generating layer is described. The charge generating layer can be formed by: applying a charge-generating-layer coating solution obtained by subjecting a charge generating substance to a dispersion treatment together with a binder resin and a solvent; and drying the resultant coat. Alternatively, the charge generating layer may be a deposited film of the charge generating substance.

Examples of the charge generating substance to be used for the charge generating layer include azo pigments, phthalocyanine pigments, indigo pigments, perylene pigments, polycyclic quinone pigments, squarylium dyes, pyrylium salts, thiapyrylium salts, triphenylmethane dyes, quinacridone pigments, azulениum salt pigments, cyanine dyestuffs, anthanthrone pigments, pyranthrone pigments, xanthene dyes, quinone imine dyes, and styryl dyes. Only one kind of those charge generating substances may be used or two or more kinds thereof may be used. Of those charge generating substances, from the viewpoint of sensitivity, phthalocyanine pigments or azo pigments are preferred, and phthalocyanine pigments are particularly more preferred.

Of the phthalocyanine pigments, in particular, oxytitanium phthalocyanines, chlorogallium phthalocyanines, or hydroxygallium phthalocyanines exhibits excellent charge genera-

## 12

tion efficiency. Further, of the hydroxygallium phthalocyanines, a hydroxygallium phthalocyanine crystal of a crystal form having peaks at Bragg angles 20 in CuK $\alpha$  characteristic X-ray diffraction of  $7.4^\circ \pm 0.3^\circ$  and  $28.2^\circ \pm 0.3^\circ$  is more preferred from the viewpoint of sensitivity.

Examples of the binder resin to be used for the charge generating layer include: polymers of vinyl compounds such as styrene, vinyl acetate, vinyl chloride, an acrylic acid ester, a methacrylic acid ester, vinylidene fluoride, and trifluoroethylene; and a polyvinyl alcohol resin, a polyvinyl acetal resin, a polycarbonate resin, a polyester resin, a polysulfone resin, a polyphenylene oxide resin, a polyurethane resin, a cellulose resin, a phenol resin, a melamine resin, a silicone resin, and an epoxy resin.

The mass ratio between the charge generating substance and the binder resin preferably falls within the range of from 1:0.3 to 1:4. As a method for the dispersion treatment, there are given, for example, methods each using a homogenizer, 15 ultrasonic dispersion, a ball mill, a vibrating ball mill, a sand mill, an attritor, or a roll mill.

Examples of the solvent to be used for the charge-generating-layer coating solution include an alcohol-based solvent, a sulfoxide-based solvent, a ketone-based solvent, an ether-based solvent, an ester-based solvent, an aliphatic halogenated hydrocarbon-based solvent, and an aromatic compound.

Next, the hole transporting layer is described. The hole transporting layer can be formed by: applying a hole-transferring-layer coating solution obtained by dissolving a hole transporting substance and a binder resin in a solvent to form a coat; and drying the resultant coat.

When the hole transporting layer is the surface layer, the hole transporting substance of the present invention is used as 35 the hole transporting substance to be used in the hole transporting layer. In addition, a known hole transporting substance can be used in addition to the hole transporting substance of the present invention. Examples of the known hole transporting substance include a carbazole compound, a hydrazone compound, an N,N-dialkylaniline compound, a diphenylamine compound, a triphenylamine compound, a triphenylmethane compound, a pyrazoline compound, a styryl compound, and a stilbene compound.

Examples of the binder resin to be used for the hole transporting layer include an acrylic acid ester, a methacrylic acid ester, a polyvinyl alcohol resin, a polyvinyl acetal resin, a polycarbonate resin, and a polyester resin. A polycarbonate resin or a polyester resin is preferred.

Examples of the solvent to be used for the hole-transferring-layer coating solution include an alcohol-based solvent, a sulfoxide-based solvent, a ketone-based solvent, an ether-based solvent, an ester-based solvent, an aliphatic halogenated hydrocarbon-based solvent, and an aromatic hydrocarbon-based solvent.

The thickness of the hole transporting layer is preferably 1  $\mu\text{m}$  or more and 50  $\mu\text{m}$  or less, more preferably 3  $\mu\text{m}$  or more and 40  $\mu\text{m}$  or less, still more preferably 5  $\mu\text{m}$  or more and 30  $\mu\text{m}$  or less.

The electrophotographic photosensitive member of the present invention may be further provided with a surface layer. In that case, the hole transporting substance of the present invention is incorporated into a protective layer.

As a binder resin to be used for the surface layer, there are given, for example, an acrylic acid ester, a methacrylic acid ester, a polyvinyl alcohol resin, a polyvinyl acetal resin, a polycarbonate resin, and a polyester resin. In addition, the surface layer may also contain a curable resin. As the curable

## 13

resin, there may be used a curable phenol resin, a curable epoxy resin, a curable acrylic resin, a curable methacrylic resin, or the like.

The surface layer can be formed by: applying a surface-layer coating solution obtained by dissolving the resin in an organic solvent to form a coat; and drying the resultant coat. The thickness of the surface layer is preferably 0.1  $\mu\text{m}$  or more and 30  $\mu\text{m}$  or less, more preferably 0.5  $\mu\text{m}$  or more and 15  $\mu\text{m}$  or less. Examples of the solvent to be used for the surface-layer coating solution include an alcohol-based solvent, a sulfoxide-based solvent, a ketone-based solvent, an ether-based solvent, an ester-based solvent, an aliphatic halogenated hydrocarbon-based solvent, and an aromatic hydrocarbon-based solvent.

In addition, the following known particles or lubricant may be incorporated into the surface layer of the electrophotographic photosensitive member: conductive particles, silicone oil, wax, fluorine atom-containing resin particles such as polytetrafluoroethylene particles, silica particles, alumina particles, boron nitride, or the like.

Any of various additives may be added to each of the layers of the electrophotographic photosensitive member. Examples of the additives include: antidegradants such as an antioxidant and a UV absorber; a coating property improving agents such as a leveling agent; organic resin particles such as fluorine atom-containing resin particles and acrylic resin particles; and inorganic particles of, for example, silica, titanium oxide, and alumina.

In the application of the coating solution for each of the layers, there may be used any known application method such as a dip coating method, a spray coating method, a ring coating method, a spin coating method, a roller coating method, a Mayer bar coating method, or a blade coating method.

Next, FIG. 4 and FIG. 5 illustrate examples of the constructions of an electrophotographic apparatus and a process cartridge each including the electrophotographic photosensitive member of the present invention, respectively.

FIG. 4 illustrates an example of the electrophotographic apparatus. Transfer paper 11 as a medium to be output is held in a sheet feeding tray 13 and is conveyed to a secondary transferring device 14 through a sheet feeding path 12. After a secondary transfer step, image fixation is performed with a fixing device 15, and the transfer paper 11 is output from a sheet delivery portion 16. The following process cartridges, which are placed side by side along an intermediate transfer member 10, each represent a process cartridge for each color to be used for color printing: a process cartridge 17 for a yellow color, a process cartridge 18 for a magenta color, a process cartridge 19 for a cyan color, and a process cartridge 20 for a black color, corresponding to respective colors, i.e., a yellow color, a magenta color, a cyan color, and a black color. The process cartridge is illustrated in detail in FIG. 5.

In FIG. 5, a cylindrical electrophotographic photosensitive member 1 is rotationally driven about its central axis in a

## 14

direction indicated by an arrow at a predetermined peripheral speed. The peripheral surface of the electrophotographic photosensitive member 1 to be rotationally driven is uniformly charged to a predetermined positive or negative potential by a charging device (primary charging device: a charging roller or the like) 2. A voltage to be applied to the charging device 2 may be any one of a voltage obtained by superimposing an AC component on a DC component, and a voltage consisting of the DC component. The charged peripheral surface of the electrophotographic photosensitive member 1 receives exposure light (image exposure light) 3 output from an exposing device (not shown) such as slit exposure or laser beam scanning exposure. Thus, electrostatic latent images corresponding to a target image are sequentially formed on the peripheral surface of the electrophotographic photosensitive member 1. The electrostatic latent images formed on the peripheral surface of the electrophotographic photosensitive member 1 are developed with toner in the developer of a developing device 4 to be turned into toner images. The toner images formed and supported on the peripheral surface of the electrophotographic photosensitive member 1 are sequentially transferred onto a transfer material (such as an intermediate transfer member) 6 by a transfer bias from a transferring device (such as a transfer roller) 5. The surface of the electrophotographic photosensitive member 1 after the transfer of the toner images is subjected to an electricity eliminating treatment with electricity eliminating light 7 from an electricity eliminating light irradiation device (not shown), and is then cleaned through the removal of transfer residual toner by a cleaning device 8. Thus, the electrophotographic photosensitive member 1 is repeatedly used in image formation. It should be noted that the electricity eliminating light irradiation step may be operated before or after a cleaning step. The electricity eliminating light irradiation device and the cleaning device 8 can be provided as required.

40 FIG. 4 illustrates a state where those devices and the like are integrally supported to form a cartridge. For example, the following may be adopted: multiple components are selected from the components such as the electrophotographic photosensitive member 1, the charging device 2, the developing device 4, and the cleaning device 8, and are 45 integrally supported to form a process cartridge, and the process cartridge can be detachably mountable to the main body of the electrophotographic apparatus. In FIG. 5, the electrophotographic photosensitive member 1, the charging device 2, the developing device 4, and the cleaning device 8 are 50 integrally supported to form a cartridge. Then, the cartridge is used as a process cartridge 9 detachably mountable to the main body of the electrophotographic apparatus.

Next, preferred examples of the hole transporting substance of the present invention are shown; provided that the present invention is not limited thereto.

No. 1



No. 2



**15****16**

-continued

No. 3



No. 4

No. 5



No. 6



No. 7



No. 8



No. 9



No. 10



No. 11



No. 12



No. 13



No. 14



17

-continued  
No. 15

18



No. 16

No. 17



No. 19



No. 21



No. 23



No. 20



No. 22



No. 24



**19**

-continued

No. 25

**20**

No. 26



No. 27



No. 28



No. 29



No. 30



No. 31



No. 32



No. 33



No. 34

21



22

-continued  
No. 35

No. 36



No. 37



No. 38



No. 39

No. 40



No. 41



No. 42



No. 43



No. 44



23



24

-continued  
No. 45

No. 46



No. 47

No. 48



No. 49



No. 50

No. 51



No. 52



No. 52



No. 54



No. 54



No. 55

**25****26**-continued  
No. 56

No. 57

No. 58



No. 59



No. 60



-continued

No. 61



No. 62



No. 63



No. 64



No. 65



No. 66



No. 67



29

30

-continued



No. 68



No. 69

No. 70



No. 71



No. 72



No. 73

31



32

-continued  
No. 74

No. 75

No. 76



No. 77



No. 78



No. 79



No. 80



No. 81



No. 82



33

34

-continued

No. 83



No. 84



No. 85



No. 86



No. 87



No. 88



No. 89



No. 90



**35**

-continued  
No. 91

**36**

No. 92

No. 93



No. 94



No. 95



No. 96



No. 97



No. 98



No. 99

37



38

-continued  
No. 100

No. 101



No. 102



No. 103

No. 104



No. 105

No. 106



-continued

No. 107



No. 108



No. 109



No. 110



No. 111



No. 112



No. 113



**41****42**

-continued

No. 114



No. 115



No. 116



No. 117



No. 118



No. 119



**43****44**

-continued

No. 120

No. 121



No. 122



No. 123

No. 124



**45****46**

-continued

No. 125

No. 126



No. 127



No. 128



-continued

No. 129



No. 130



**49****50**

-continued

No. 131



No. 132



No. 133





-continued

No. 137



No. 138



No. 139



**55****56**

-continued

No. 140

No. 141



No. 142



-continued

No. 143



No. 144



No. 145



59

60

-continued



No. 146



No. 147



No. 148



**61****62**

-continued

No. 149

No. 150



No. 151



No. 152



No. 153



No. 154



No. 155



No. 156



No. 157

-continued

No. 158



No. 159



No. 160



No. 161

No. 162



No. 163

No. 164



No. 165

No. 166



No. 167



**65****66**

-continued

No. 168



No. 169



No. 170



No. 171



No. 172



No. 173



No. 174





No. 176



No. 178



No. 180



No. 182



No. 183



No. 184



**69****70**

-continued

No. 185

No. 186



No. 187

No. 188



No. 189



No. 190



No. 191





-continued

No. 192



No. 193

No. 194



No. 195



No. 196



No. 197



No. 198



-continued

No. 199



No. 200



No. 201



No. 202



No. 203





No. 205

-continued



No. 204



No. 206



No. 207



No. 208



No. 209



No. 210

No. 211

-continued

No. 212



No. 213



No. 214



No. 215



No. 216



79

80

-continued

No. 217



No. 218



No. 219



No. 220

No. 221



-continued

No. 222



No. 223



No. 224

No. 225



No. 226

No. 227



No. 228

No. 228



83

84

-continued

No. 229



No. 230



No. 231



No. 232



85

86

-continued

No. 233



No. 234



No. 235



No. 236





89

90

-continued

No. 241



No. 242



No. 243



91

92

-continued  
No. 244



No. 245

No. 246



No. 247

No. 248



No. 249



No. 250



93

94

-continued



No. 251



No. 252



No. 253



No. 254

-continued

No. 255



No. 256



No. 257



97



98



-continued

No. 258

No. 259



No. 260



No. 261



No. 262

-continued

No. 263



No. 264



No. 265



No. 266



101

-continued



102

No. 267



No. 268



No. 269

-continued



A representative synthesis example of the hole transporting substance to be used in the present invention is described below.

Exemplified Compound No. 56 was synthesized by a reaction represented by the following reaction formula [1]. A three-necked flask was mounted with a nitrogen introducing tube, a cooling tube, an inner temperature gauge, and the like. 30  
 350 Parts of toluene, 160 parts of ethanol, and 200 parts of a 10-mass % aqueous solution of sodium carbonate were mixed, and nitrogen replacement was performed by stirring the mixture with a mechanical stirrer for 30 minutes or more at room temperature well while performing nitrogen gas bubbling. Further, 22.4 parts of 1-boronic acid pinacol ester-7-  
 40  
 45  
 50  
 55  
 60  
 65  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350  
 355  
 360  
 365  
 370  
 375  
 380  
 385  
 390  
 395  
 400  
 405  
 410  
 415  
 420  
 425  
 430  
 435  
 440  
 445  
 450  
 455  
 460  
 465  
 470  
 475  
 480  
 485  
 490  
 495  
 500  
 505  
 510  
 515  
 520  
 525  
 530  
 535  
 540  
 545  
 550  
 555  
 560  
 565  
 570  
 575  
 580  
 585  
 590  
 595  
 600  
 605  
 610  
 615  
 620  
 625  
 630  
 635  
 640  
 645  
 650  
 655  
 660  
 665  
 670  
 675  
 680  
 685  
 690  
 695  
 700  
 705  
 710  
 715  
 720  
 725  
 730  
 735  
 740  
 745  
 750  
 755  
 760  
 765  
 770  
 775  
 780  
 785  
 790  
 795  
 800  
 805  
 810  
 815  
 820  
 825  
 830  
 835  
 840  
 845  
 850  
 855  
 860  
 865  
 870  
 875  
 880  
 885  
 890  
 895  
 900  
 905  
 910  
 915  
 920  
 925  
 930  
 935  
 940  
 945  
 950  
 955  
 960  
 965  
 970  
 975  
 980  
 985  
 990  
 995  
 1000  
 1005  
 1010  
 1015  
 1020  
 1025  
 1030  
 1035  
 1040  
 1045  
 1050  
 1055  
 1060  
 1065  
 1070  
 1075  
 1080  
 1085  
 1090  
 1095  
 1100  
 1105  
 1110  
 1115  
 1120  
 1125  
 1130  
 1135  
 1140  
 1145  
 1150  
 1155  
 1160  
 1165  
 1170  
 1175  
 1180  
 1185  
 1190  
 1195  
 1200  
 1205  
 1210  
 1215  
 1220  
 1225  
 1230  
 1235  
 1240  
 1245  
 1250  
 1255  
 1260  
 1265  
 1270  
 1275  
 1280  
 1285  
 1290  
 1295  
 1300  
 1305  
 1310  
 1315  
 1320  
 1325  
 1330  
 1335  
 1340  
 1345  
 1350  
 1355  
 1360  
 1365  
 1370  
 1375  
 1380  
 1385  
 1390  
 1395  
 1400  
 1405  
 1410  
 1415  
 1420  
 1425  
 1430  
 1435  
 1440  
 1445  
 1450  
 1455  
 1460  
 1465  
 1470  
 1475  
 1480  
 1485  
 1490  
 1495  
 1500  
 1505  
 1510  
 1515  
 1520  
 1525  
 1530  
 1535  
 1540  
 1545  
 1550  
 1555  
 1560  
 1565  
 1570  
 1575  
 1580  
 1585  
 1590  
 1595  
 1600  
 1605  
 1610  
 1615  
 1620  
 1625  
 1630  
 1635  
 1640  
 1645  
 1650  
 1655  
 1660  
 1665  
 1670  
 1675  
 1680  
 1685  
 1690  
 1695  
 1700  
 1705  
 1710  
 1715  
 1720  
 1725  
 1730  
 1735  
 1740  
 1745  
 1750  
 1755  
 1760  
 1765  
 1770  
 1775  
 1780  
 1785  
 1790  
 1795  
 1800  
 1805  
 1810  
 1815  
 1820  
 1825  
 1830  
 1835  
 1840  
 1845  
 1850  
 1855  
 1860  
 1865  
 1870  
 1875  
 1880  
 1885  
 1890  
 1895  
 1900  
 1905  
 1910  
 1915  
 1920  
 1925  
 1930  
 1935  
 1940  
 1945  
 1950  
 1955  
 1960  
 1965  
 1970  
 1975  
 1980  
 1985  
 1990  
 1995  
 2000  
 2005  
 2010  
 2015  
 2020  
 2025  
 2030  
 2035  
 2040  
 2045  
 2050  
 2055  
 2060  
 2065  
 2070  
 2075  
 2080  
 2085  
 2090  
 2095  
 2100  
 2105  
 2110  
 2115  
 2120  
 2125  
 2130  
 2135  
 2140  
 2145  
 2150  
 2155  
 2160  
 2165  
 2170  
 2175  
 2180  
 2185  
 2190  
 2195  
 2200  
 2205  
 2210  
 2215  
 2220  
 2225  
 2230  
 2235  
 2240  
 2245  
 2250  
 2255  
 2260  
 2265  
 2270  
 2275  
 2280  
 2285  
 2290  
 2295  
 2300  
 2305  
 2310  
 2315  
 2320  
 2325  
 2330  
 2335  
 2340  
 2345  
 2350  
 2355  
 2360  
 2365  
 2370  
 2375  
 2380  
 2385  
 2390  
 2395  
 2400  
 2405  
 2410  
 2415  
 2420  
 2425  
 2430  
 2435  
 2440  
 2445  
 2450  
 2455  
 2460  
 2465  
 2470  
 2475  
 2480  
 2485  
 2490  
 2495  
 2500  
 2505  
 2510  
 2515  
 2520  
 2525  
 2530  
 2535  
 2540  
 2545  
 2550  
 2555  
 2560  
 2565  
 2570  
 2575  
 2580  
 2585  
 2590  
 2595  
 2600  
 2605  
 2610  
 2615  
 2620  
 2625  
 2630  
 2635  
 2640  
 2645  
 2650  
 2655  
 2660  
 2665  
 2670  
 2675  
 2680  
 2685  
 2690  
 2695  
 2700  
 2705  
 2710  
 2715  
 2720  
 2725  
 2730  
 2735  
 2740  
 2745  
 2750  
 2755  
 2760  
 2765  
 2770  
 2775  
 2780  
 2785  
 2790  
 2795  
 2800  
 2805  
 2810  
 2815  
 2820  
 2825  
 2830  
 2835  
 2840  
 2845  
 2850  
 2855  
 2860  
 2865  
 2870  
 2875  
 2880  
 2885  
 2890  
 2895  
 2900  
 2905  
 2910  
 2915  
 2920  
 2925  
 2930  
 2935  
 2940  
 2945  
 2950  
 2955  
 2960  
 2965  
 2970  
 2975  
 2980  
 2985  
 2990  
 2995  
 3000  
 3005  
 3010  
 3015  
 3020  
 3025  
 3030  
 3035  
 3040  
 3045  
 3050  
 3055  
 3060  
 3065  
 3070  
 3075  
 3080  
 3085  
 3090  
 3095  
 3100  
 3105  
 3110  
 3115  
 3120  
 3125  
 3130  
 3135  
 3140  
 3145  
 3150  
 3155  
 3160  
 3165  
 3170  
 3175  
 3180  
 3185  
 3190  
 3195  
 3200  
 3205  
 3210  
 3215  
 3220  
 3225  
 3230  
 3235  
 3240  
 3245  
 3250  
 3255  
 3260  
 3265  
 3270  
 3275  
 3280  
 3285  
 3290  
 3295  
 3300  
 3305  
 3310  
 3315  
 3320  
 3325  
 3330  
 3335  
 3340  
 3345  
 3350  
 3355  
 3360  
 3365  
 3370  
 3375  
 3380  
 3385  
 3390  
 3395  
 3400  
 3405  
 3410  
 3415  
 3420  
 3425  
 3430  
 3435  
 3440  
 3445  
 3450  
 3455  
 3460  
 3465  
 3470  
 3475  
 3480  
 3485  
 3490  
 3495  
 3500  
 3505  
 3510  
 3515  
 3520  
 3525  
 3530  
 3535  
 3540  
 3545  
 3550  
 3555  
 3560  
 3565  
 3570  
 3575  
 3580  
 3585  
 3590  
 3595  
 3600  
 3605  
 3610  
 3615  
 3620  
 3625  
 3630  
 3635  
 3640  
 3645  
 3650  
 3655  
 3660  
 3665  
 3670  
 3675  
 3680  
 3685  
 3690  
 3695  
 3700  
 3705  
 3710  
 3715  
 3720  
 3725  
 3730  
 3735  
 3740  
 3745  
 3750  
 3755  
 3760  
 3765  
 3770  
 3775  
 3780  
 3785  
 3790  
 3795  
 3800  
 3805  
 3810  
 3815  
 3820  
 3825  
 3830  
 3835  
 3840  
 3845  
 3850  
 3855  
 3860  
 3865  
 3870  
 3875  
 3880  
 3885  
 3890  
 3895  
 3900  
 3905  
 3910  
 3915  
 3920  
 3925  
 3930  
 3935  
 3940  
 3945  
 3950  
 3955  
 3960  
 3965  
 3970  
 3975  
 3980  
 3985  
 3990  
 3995  
 4000  
 4005  
 4010  
 4015  
 4020  
 4025  
 4030  
 4035  
 4040  
 4045  
 4050  
 4055  
 4060  
 4065  
 4070  
 4075  
 4080  
 4085  
 4090  
 4095  
 4100  
 4105  
 4110  
 4115  
 4120  
 4125  
 4130  
 4135  
 4140  
 4145  
 4150  
 4155  
 4160  
 4165  
 4170  
 4175  
 4180  
 4185  
 4190  
 4195  
 4200  
 4205  
 4210  
 4215  
 4220  
 4225  
 4230  
 4235  
 4240  
 4245  
 4250  
 4255  
 4260  
 4265  
 4270  
 4275  
 4280  
 4285  
 4290  
 4295  
 4300  
 4305  
 4310  
 4315  
 4320  
 4325  
 4330  
 4335  
 4340  
 4345  
 4350  
 4355  
 4360  
 4365  
 4370  
 4375  
 4380  
 4385  
 4390  
 4395  
 4400  
 4405  
 4410  
 4415  
 4420  
 4425  
 4430  
 4435  
 4440  
 4445  
 4450  
 4455  
 4460  
 4465  
 4470  
 4475  
 4480  
 4485  
 4490  
 4495  
 4500  
 4505  
 4510  
 4515  
 4520  
 4525  
 4530  
 4535  
 4540  
 4545  
 4550  
 4555  
 4560  
 4565  
 4570  
 4575  
 4580  
 4585  
 4590  
 4595  
 4600  
 4605  
 4610  
 4615  
 4620  
 4625  
 4630  
 4635  
 4640  
 4645  
 4650  
 4655  
 4660  
 4665  
 4670  
 4675  
 4680  
 4685  
 4690  
 4695  
 4700  
 4705  
 4710  
 4715  
 4720  
 4725  
 4730  
 4735  
 4740  
 4745  
 4750  
 4755  
 4760  
 4765  
 4770  
 4775  
 4780  
 4785  
 4790  
 4795  
 4800  
 4805  
 4810  
 4815  
 4820  
 4825  
 4830  
 4835  
 4840  
 4845  
 4850  
 4855  
 4860  
 4865  
 4870  
 4875  
 4880  
 4885  
 4890  
 4895  
 4900  
 4905  
 4910  
 4915  
 4920  
 4925  
 4930  
 4935  
 4940  
 4945  
 4950  
 4955  
 4960  
 4965  
 4970  
 4975  
 4980  
 4985  
 4990  
 4995  
 5000  
 5005  
 5010  
 5015  
 5020  
 5025  
 5030  
 5035  
 5040  
 5045  
 5050  
 5055  
 5060  
 5065  
 5070  
 5075  
 5080  
 5085  
 5090  
 5095  
 5100  
 5105  
 5110  
 5115  
 5120  
 5125  
 5130  
 5135  
 5140  
 5145  
 5150  
 5155  
 5160  
 5165  
 5170  
 5175  
 5180  
 5185  
 5190  
 5195  
 5200  
 5205  
 5210  
 5215  
 5220  
 5225  
 5230  
 5235  
 5240  
 5245  
 5250  
 5255  
 5260  
 5265  
 5270  
 5275  
 5280  
 5285  
 5290  
 5295  
 5300  
 5305  
 5310  
 5315  
 5320  
 5325  
 5330  
 5335  
 5340  
 5345  
 5350  
 5355  
 5360  
 5365  
 5370  
 5375  
 5380  
 5385  
 5390  
 5395  
 5400  
 5405  
 5410  
 5415  
 5420  
 5425  
 5430  
 5435  
 5440  
 5445  
 5450  
 5455  
 5460  
 5465  
 5470  
 5475  
 5480  
 5485  
 5490  
 5495  
 5500  
 5505  
 5510  
 5515  
 5520  
 5525  
 5530  
 5535  
 5540  
 5545  
 5550  
 5555  
 5560  
 5565  
 5570  
 5575  
 5580  
 5585  
 5590  
 5595  
 5600  
 5605  
 5610  
 5615  
 5620  
 5625  
 5630  
 5635  
 5640  
 5645  
 5650  
 5655  
 5660  
 5665  
 5670  
 5675  
 5680  
 5685  
 5690  
 5695  
 5700  
 5705  
 5710  
 5715  
 5720  
 5725  
 5730  
 5735  
 5740  
 5745  
 5750  
 5755  
 5760  
 5765  
 5770  
 5775  
 5780  
 5785  
 5790  
 5795  
 5800  
 5805  
 5810  
 5815  
 5820  
 5825  
 5830  
 5835  
 5840  
 5845  
 5850  
 5855  
 5860  
 5865  
 5870  
 5875  
 5880  
 5885  
 5890  
 5895  
 5900  
 5905  
 5910  
 5915  
 5920  
 5925  
 5930  
 5935  
 5940  
 5945  
 5950  
 5955  
 5960  
 5965  
 5970  
 5975  
 5980  
 5985  
 5990  
 5995  
 6000  
 6005  
 6010  
 6015  
 6020  
 6025  
 6030  
 6035  
 6040  
 6045  
 6050  
 6055  
 6060  
 6065  
 6070  
 6075  
 6080  
 6085  
 6090  
 6095  
 6100  
 6105  
 6110  
 6115  
 6120  
 6125  
 6130  
 6135  
 6140  
 6145  
 6150  
 6155  
 6160  
 6165  
 6170  
 6175  
 6180  
 6185  
 6190  
 6195  
 6200  
 6205  
 6210  
 6215  
 6220  
 6225  
 6230  
 6235  
 6240  
 6245  
 6250  
 6255  
 6260  
 6265  
 6270  
 6275  
 6280  
 6285  
 6290  
 6295  
 6300  
 6305  
 6310  
 6315  
 6320  
 6325  
 6330  
 6335  
 6340  
 6345  
 6350  
 6355  
 6360  
 6365  
 6370  
 6375  
 6380  
 6385  
 6390  
 6395  
 6400  
 6405  
 6410  
 6415  
 6420  
 6425  
 6430  
 6435  
 6440  
 6445  
 6450  
 6455  
 6460  
 6465  
 6470  
 6475  
 6480  
 6485  
 6490  
 6495  
 6500  
 6505  
 6510  
 6515  
 6520  
 6525  
 6530  
 6535  
 6540  
 6545  
 6550  
 6555  
 6560  
 6565  
 6570  
 6575  
 6580  
 6585  
 6590  
 6595  
 6600  
 6605  
 6610  
 6615  
 6620  
 6625  
 6630  
 6635  
 6640  
 6645  
 6650  
 6655  
 6660  
 6665  
 6670  
 6675  
 6680  
 6685  
 6690  
 6695  
 6700  
 6705  
 6710  
 6715  
 6720  
 6725  
 6730  
 6735  
 6740  
 6745  
 6750  
 6755  
 6760  
 6765  
 6770  
 6775  
 6780  
 6785  
 6790  
 6795  
 6800  
 6805  
 6810  
 6815  
 6820  
 6825  
 6830  
 6835  
 6840  
 6845  
 6850  
 6855  
 6860  
 6865  
 6870  
 6875  
 6880  
 6885  
 6890  
 6895  
 6900  
 6905  
 6910  
 6915  
 6920  
 6925  
 6930  
 6935  
 6940  
 6945  
 6950  
 6955  
 6960  
 6965  
 6970

## 105

with 500 parts of toluene by stirring, and 0.8 part of a silane coupling agent was added to the mixture, followed by stirring for 6 hours. After that, toluene was removed by distillation under reduced pressure and the residue was dried by heating

## 106

the undercoat layer by dipping to form a coat, and the resultant coat was dried by heating at a temperature of 80° C. for 15 minutes to form a charge generating layer having a thickness of 0.17  $\mu\text{m}$ .



at 130° C. for 6 hours to provide surface-treated zinc oxide particles. KBM602 (compound name: N-2-(aminoethyl)-3-aminopropylmethyldimethoxysilane) manufactured by Shin-Etsu Chemical Co., Ltd. was used as the silane coupling agent.

Next, 15 parts of a polyvinyl butyral resin (weight-average molecular weight: 40,000, trade name: BM-1, manufactured by SEKISUI CHEMICAL CO., LTD.) and 15 parts of a blocked isocyanate (trade name: Sumidur 3175, manufactured by Sumika Bayer Urethane Co., Ltd.) were dissolved in a mixed solution of 73.5 parts of methyl ethyl ketone and 73.5 parts of 1-butanol. 80.8 Parts of the surface-treated zinc oxide particles and 0.8 part of 2,3,4-trihydroxybenzophenone (manufactured by Tokyo Chemical Industry Co., Ltd.) were added to the solution, and the mixture was dispersed with a sand mill apparatus using glass beads each having a diameter of 0.8 mm under an atmosphere having a temperature of 23±3° C. for 3 hours. After the dispersion, 0.01 part of silicone oil (trade name: SH28PA, manufactured by Dow Corning Toray Co., Ltd.) and 5.6 parts of crosslinked polymethyl methacrylate (PMMA) particles (trade name: TECHPOLY-MER SSX-102, manufactured by SEKISUI PLASTICS CO., Ltd., average primary particle diameter: 2.5  $\mu\text{m}$ ) were added to the resultant, and the resultant was stirred to prepare an undercoat-layer coating solution.

The undercoat-layer coating solution was applied onto the support by dipping to form a coat, and the resultant coat was dried for 40 minutes at 160° C. to form an undercoat layer having a thickness of 18  $\mu\text{m}$ .

Next, a hydroxygallium phthalocyanine crystal (charge generating substance) of a crystal form having peaks at Bragg angles 20±0.2° in CuK $\alpha$  characteristic X-ray diffraction of 7.4° and 28.2° was prepared. 20 Parts of the hydroxygallium phthalocyanine crystal, 0.2 part of a calixarene compound represented by the following formula (3), 10 parts of a polyvinyl butyral resin (trade name: S-LEC BX-1, manufactured by SEKISUI CHEMICAL CO., LTD.), and 600 parts of cyclohexanone were dispersed with a sand mill apparatus using glass beads each having a diameter of 1 mm for 4 hours. After that, 700 parts of ethyl acetate were added to the resultant to prepare a charge-generating-layer coating solution. The charge-generating-layer coating solution was applied onto

25 Next, 60 parts of a hole transporting substance represented by the following formula (4), 20 parts of a hole transporting substance represented by the following formula (5), and 100 parts of a polycarbonate resin (Iupilon 2400 manufactured by 30 Mitsubishi Engineering-Plastics Corporation) were dissolved in a mixed solvent of 600 parts of monochlorobenzene and 200 parts of methylal to prepare a hole-transporting-layer coating solution. The hole-transporting-layer coating solution was applied onto the charge generating layer by dipping to form a coat, and the resultant coat was dried by heating at a temperature of 110° C. for 60 minutes to form a hole 35 transporting layer having a thickness of 16  $\mu\text{m}$ .



Next, 8 parts of the compound (hole transporting substance of the present invention) represented by Exemplified Compound No. 56, 10 parts of a polycarbonate resin (Iupilon 2800 manufactured by Mitsubishi Engineering-Plastics Corpora-

107

tion), 440 parts of monochlorobenzene, and 440 parts of tetrahydrofuran were mixed and stirred well. The mixture was filtered with a membrane filter to prepare a protective-layer (surface-layer) coating solution.

The protective-layer coating solution was applied onto the hole transporting layer by spraying to form a coat, and the resultant coat was dried by heating in an oven at a temperature of 110°C. for 30 minutes to form a protective layer (surface layer) having a thickness of 7 µm. The electrophotographic photosensitive member thus produced was subjected to the following evaluation.

(Evaluation of Electrophotographic Photosensitive Member)

A photosensitive member testing apparatus (CYNTHIA 59 manufactured by GEN-TECH, INC.) was used in the evaluation of the electrophotographic photosensitive member for its initial sensitivity and residual potential. First, a condition for a charging device was set so that the dark-area potential (Vd) of the electrophotographic photosensitive member became -700 (V) under a 23°C./50% RH environment. The photosensitive member was irradiated with monochromatic light having a wavelength of 780 nm, and the quantity of the light needed for reducing the potential of -700 (V) to -200 (V) was measured and defined as a sensitivity  $\Delta 500$  ( $\mu\text{J}/\text{cm}^2$ ). Further, the potential of the electrophotographic photosensitive member when the photosensitive member was irradiated with light having a quantity of 20 ( $\mu\text{J}/\text{cm}^2$ ) was measured as a residual potential Vr (-V).

The produced electrophotographic photosensitive member was mounted onto the cyan station of a reconstructed machine of an electrophotographic copying machine (trade name: iR-ADV C5051) manufactured by Canon Inc. as an image evaluating apparatus, and was evaluated as described below.

First, a condition for a charging device was set so that the dark-area potential (Vd) of the electrophotographic photosensitive member became -700 (V) under a 23°C./50% RH environment. The photosensitive member was irradiated with laser light having a wavelength of 780 nm, the quantity of the light needed for reducing the potential of -700 (V) to -200 (V) was determined, and repeated image formation was performed by continuously outputting an evaluation chart, which was an A4 horizontal 5% image, on 5,000 sheets. The image formation was performed by reconstructing the electrophotographic apparatus so that the total quantity of a discharge current in its charging step became 300 ( $\mu\text{A}$ ).

After the completion of the repeated image formation, the electrophotographic photosensitive member taken out of the image evaluating apparatus was immediately mounted onto the same photosensitive member testing apparatus as that described above, its sensitivity and residual potential were measured, and a variation between potentials before and after the repeated image formation was evaluated.

Next, an apparatus reconstructed so as to be capable of, for example, regulation and measurement so that image exposure laser power, the quantity of a current flowing from a charging roller to a support (hereinafter described as "total current"), and the DC component and AC component of a voltage to be applied to the charging roller could each be controlled was prepared as an electrophotographic apparatus. In addition, evaluation was performed while the power source of a heater accompanying the main body of the electrophotographic apparatus was turned off.

A cyan cartridge to be used in the electrophotographic apparatus was prepared, and the electrophotographic apparatus, the cartridge, and the electrophotographic photosensitive member were left to stand under a 30°C./80% RH environment for 24 hours or more. After that, the electrophotographic photosensitive member was mounted onto the cyan cartridge for image formation and evaluation. Then, an entire exposure image having a cyan color alone was output on A4 size plain

108

paper and an image exposure light quantity was set so that a density on the paper measured with a spectral densitometer (trade name: X-Rite 504, manufactured by X-Rite Inc.) became 1.45.

Evaluation for image reproducibility was performed by setting the total quantity of a discharge current in the step of charging the electrophotographic photosensitive member to 300 ( $\mu\text{A}$ ). A 5,000-sheet repeated image formation test was performed with a test chart having an image density ratio of 5% in this setting. After the completion of the repeated image formation, the electrophotographic photosensitive member was taken out of the electrophotographic apparatus together with the cartridge, and was left to stand under the same 30°C./80% RH environment in a dark place for 24 hours.

After that, the cartridge including the electrophotographic photosensitive member was mounted onto the same electrophotographic apparatus again, and an A4 horizontal 1-dot/1-space image having an output resolution of 600 dpi was formed. Then, the output image was visually observed, and image reproducibility on entire A4 paper in which image deletion was involved was evaluated by the following criteria.

Evaluation ranks were as described below.

<A>: When dots of the image are magnified and observed, none of the disturbance and scattering of the dots is present (that is, the image deletion is absent), and hence the image reproducibility is good.

<B>: When dots of the image are magnified and observed, the disturbance of part of the dots is observed but the scattering thereof is absent.

<C>: When dots of the image are magnified and observed, the disturbance, scattering, and disappearance of part of the dots occur.

<D>: When dots of the image are magnified and observed, the disturbance, scattering, and disappearance of the entire dots occur.

<E>: When dots of the image are magnified and observed, white voids occur on the image and hence the image reproducibility is low (the image deletion occurs on the entire image).

Table 1 shows the result of the evaluation for the electric potential variation due to repeated image formation, and the results of the evaluation for image characteristics under a high-temperature and high-humidity environment.

#### Examples 2 to 18

Electrophotographic photosensitive members were each produced and evaluated in the same manner as in Example 1 except that the hole transporting substance used in the protective layer of Example 1 was changed to a hole transporting substance shown in Table 1. Table 1 shows the results of the evaluation.

#### Example 19

The hole transporting substance used in the protective layer of Example 1 was changed as follows: 7.2 parts of the hole transporting substance represented by Exemplified Compound No. 56 and 0.8 part of the hole transporting substance represented by the formula (5) were used as a mixture. Further, 10 parts of the same polycarbonate resin as that of Example 1, 440 parts of monochlorobenzene, and 440 parts of tetrahydrofuran were mixed to prepare a protective-layer coating solution. A protective layer was formed and an electrophotographic photosensitive member was produced in the same manner as in Example 1 except the foregoing. Further, the electrophotographic photosensitive member was evaluated in the same manner as in Example 1. Table 1 shows the results of the evaluation.

#### Example 20

The hole transporting substance used in the protective layer of Example 1 was changed as follows: 6.4 parts of the hole

## 109

transporting substance represented by Exemplified Compound No. 56 and 1.6 parts of the hole transporting substance represented by the formula (5) were used as a mixture. Further, 10 parts of the same polycarbonate resin as that of Example 1, 440 parts of monochlorobenzene, and 440 parts of tetrahydrofuran were mixed to prepare a protective-layer coating solution. A protective layer was formed and an electrophotographic photosensitive member was produced in the same manner as in Example 1 except the foregoing. Further, the electrophotographic photosensitive member was evaluated in the same manner as in Example 1. Table 1 shows the results of the evaluation.

## Example 21

The hole transporting substance used in the surface layer of Example 1 was changed as follows: 4 parts of the hole transporting substance represented by Exemplified Compound No. 56 and 4 parts of the hole transporting substance represented by the formula (5) were used as a mixture. Further, 10 parts of the same polycarbonate resin as that of Example 1, 440 parts of monochlorobenzene, and 440 parts of tetrahydrofuran were mixed to prepare a protective-layer coating solution. An electrophotographic photosensitive member was produced in the same manner as in Example 1 except the foregoing. Further, the electrophotographic photosensitive member was evaluated in the same manner as in Example 1. Table 1 shows the results of the evaluation.

## Example 22

An electrophotographic photosensitive member was produced and evaluated in the same manner as in Example 1 except that the hole transporting substance used in the protective layer of Example 1 was changed to a hole transporting substance shown in Table 1. Table 1 shows the results of the evaluation.

## Comparative Example 1

An electrophotographic photosensitive member was produced in the same manner as in Example 1 except that the hole transporting substance used in the protective layer of Example 1 was changed to a hole transporting substance represented by the following formula (6), and the electrophotographic photosensitive member was similarly evaluated. Table 1 shows the results of the evaluation.



## Comparative Example 2

An electrophotographic photosensitive member was produced in the same manner as in Example 1 except that the hole transporting substance used in the protective layer of

## 110

Example 1 was changed to a hole transporting substance represented by the following formula (7), and the electrophotographic photosensitive member was similarly evaluated. Table 1 shows the results of the evaluation.



## Comparative Example 3

An electrophotographic photosensitive member was produced in the same manner as in Example 1 except that the hole transporting substance used in the protective layer of Example 1 was changed to an aromatic compound represented by the following formula (8), and the electrophotographic photosensitive member was similarly evaluated. Table 1 shows the results of the evaluation.



## Comparative Example 4

An electrophotographic photosensitive member was produced in the same manner as in Example 1 except that the hole transporting substance used in the protective layer of Example 1 was changed to an aromatic compound represented by the following formula (9), and the electrophotographic photosensitive member was similarly evaluated. Table 1 shows the results of the evaluation.



## Comparative Example 5

An electrophotographic photosensitive member was produced in the same manner as in Example 1 except that the hole transporting substance used in the surface layer of Example 1 was changed to poly(9,9-diethyl-9H-fluorene-2,7-diylium) represented by the following formula (10) (manufactured by TOSCO CO., LTD., polyfluorene compound; average

## 111

molecular weight: 40,000), and the electrophotographic photosensitive member was similarly evaluated. Table 1 shows the results of the evaluation.



Comparative Example 6

An electrophotographic photosensitive member was produced in the same manner as in Example 1 except that the hole transporting substance used in the protective layer of Example 1 was changed to an aromatic compound represented by the following formula (11), and the electrophotographic photosensitive member was similarly evaluated. Table 1 shows the results of the evaluation.



Comparative Example 7

An electrophotographic photosensitive member was produced in the same manner as in Example 1 except that the hole transporting substance used in the protective layer of

## 112

Example 1 was changed to a compound represented by the following formula (12), and the electrophotographic photosensitive member was similarly evaluated. Table 1 shows the results of the evaluation.



Comparative Example 8

An electrophotographic photosensitive member was produced in the same manner as in Example 1 except that the hole transporting substance used in the protective layer of Example 1 was changed to a compound represented by the following formula (13), and the electrophotographic photosensitive member was similarly evaluated. Table 1 shows the results of the evaluation.



TABLE 1

| No.        | Kind of compound         | Hole transporting substance                                  |                                           |                                           | Initial potential at 23°C./50% RH      |                         |                                        | Potential after 5,000-sheet |  |  | 5,000-Sheet<br>endurance under high temperature<br>and high humidity<br>Image evaluation |  |
|------------|--------------------------|--------------------------------------------------------------|-------------------------------------------|-------------------------------------------|----------------------------------------|-------------------------|----------------------------------------|-----------------------------|--|--|------------------------------------------------------------------------------------------|--|
|            |                          | Number of sp <sup>2</sup> carbon atoms that form conjugation | Ratio of sp <sup>2</sup> carbon atoms (%) | Ratio of sp <sup>3</sup> carbon atoms (%) | Sensitivity Δ500 (μJ/cm <sup>2</sup> ) | Residual potential (-V) | Sensitivity Δ500 (μJ/cm <sup>2</sup> ) | Residual potential (-V)     |  |  |                                                                                          |  |
|            |                          |                                                              |                                           |                                           |                                        |                         |                                        |                             |  |  |                                                                                          |  |
| Example 1  | Exemplified Compound 56  | 44                                                           | 80                                        | 20                                        | 0.25                                   | 60                      | 0.26                                   | 64                          |  |  | A                                                                                        |  |
| Example 2  | Exemplified Compound 15  | 28                                                           | 80                                        | 20                                        | 0.29                                   | 63                      | 0.31                                   | 67                          |  |  | A                                                                                        |  |
| Example 3  | Exemplified Compound 40  | 36                                                           | 71                                        | 29                                        | 0.31                                   | 65                      | 0.32                                   | 68                          |  |  | A                                                                                        |  |
| Example 4  | Exemplified Compound 42  | 36                                                           | 61                                        | 39                                        | 0.36                                   | 73                      | 0.39                                   | 79                          |  |  | A                                                                                        |  |
| Example 5  | Exemplified Compound 44  | 36                                                           | 55                                        | 45                                        | 0.38                                   | 79                      | 0.40                                   | 86                          |  |  | B                                                                                        |  |
| Example 6  | Exemplified Compound 57  | 44                                                           | 77                                        | 23                                        | 0.26                                   | 63                      | 0.27                                   | 69                          |  |  | A                                                                                        |  |
| Example 7  | Exemplified Compound 58  | 44                                                           | 75                                        | 25                                        | 0.28                                   | 65                      | 0.28                                   | 69                          |  |  | A                                                                                        |  |
| Example 8  | Exemplified Compound 63  | 40                                                           | 80                                        | 20                                        | 0.26                                   | 62                      | 0.27                                   | 68                          |  |  | A                                                                                        |  |
| Example 9  | Exemplified Compound 66  | 40                                                           | 69                                        | 31                                        | 0.29                                   | 69                      | 0.31                                   | 74                          |  |  | A                                                                                        |  |
| Example 10 | Exemplified Compound 78  | 38                                                           | 81                                        | 19                                        | 0.28                                   | 68                      | 0.29                                   | 70                          |  |  | A                                                                                        |  |
| Example 11 | Exemplified Compound 82  | 38                                                           | 86                                        | 14                                        | 0.32                                   | 62                      | 0.34                                   | 66                          |  |  | A                                                                                        |  |
| Example 12 | Exemplified Compound 90  | 38                                                           | 88                                        | 12                                        | 0.31                                   | 67                      | 0.35                                   | 84                          |  |  | A                                                                                        |  |
| Example 13 | Exemplified Compound 108 | 36                                                           | 57                                        | 43                                        | 0.37                                   | 77                      | 0.39                                   | 82                          |  |  | B                                                                                        |  |
| Example 14 | Exemplified Compound 112 | 48                                                           | 63                                        | 37                                        | 0.34                                   | 66                      | 0.35                                   | 70                          |  |  | A                                                                                        |  |
| Example 15 | Exemplified Compound 125 | 50                                                           | 81                                        | 19                                        | 0.30                                   | 60                      | 0.32                                   | 67                          |  |  | A                                                                                        |  |
| Example 16 | Exemplified Compound 146 | 108                                                          | 58                                        | 42                                        | 0.47                                   | 85                      | 0.52                                   | 94                          |  |  | B                                                                                        |  |
| Example 17 | Exemplified Compound 166 | 36                                                           | 78                                        | 22                                        | 0.40                                   | 56                      | 0.45                                   | 67                          |  |  | B                                                                                        |  |
| Example 18 | Exemplified Compound 177 | 40                                                           | 82                                        | 18                                        | 0.36                                   | 55                      | 0.38                                   | 65                          |  |  | A                                                                                        |  |
| Example 19 | Exemplified Compound 56  | 44                                                           | 80                                        | 20                                        | 0.26                                   | 69                      | 0.30                                   | 83                          |  |  | A                                                                                        |  |

TABLE 1-continued

| No.                   | Kind of compound        | Hole transporting substance                                  |                                           |                                           | Initial potential at 23°C./50% RH      |                         | Potential after 5,000-sheet            |                         | endurance under high temperature and high humidity Image evaluation |
|-----------------------|-------------------------|--------------------------------------------------------------|-------------------------------------------|-------------------------------------------|----------------------------------------|-------------------------|----------------------------------------|-------------------------|---------------------------------------------------------------------|
|                       |                         | Number of sp <sup>2</sup> carbon atoms that form conjugation | Ratio of sp <sup>2</sup> carbon atoms (%) | Ratio of sp <sup>3</sup> carbon atoms (%) | Sensitivity Δ500 (μJ/cm <sup>2</sup> ) | Residual potential (-V) | Sensitivity Δ500 (μJ/cm <sup>2</sup> ) | Residual potential (-V) |                                                                     |
|                       |                         |                                                              |                                           |                                           |                                        |                         |                                        |                         |                                                                     |
| Example 20            | Exemplified Compound 56 | 44                                                           | 80                                        | 20                                        | 0.28                                   | 76                      | 0.37                                   | 88                      | B                                                                   |
| Example 21            | Exemplified Compound 56 | 44                                                           | 80                                        | 20                                        | 0.35                                   | 84                      | 0.41                                   | 101                     | D                                                                   |
| Example 22            | Exemplified Compound 36 | 36                                                           | 77                                        | 23                                        | 0.35                                   | 65                      | 0.38                                   | 87                      | C                                                                   |
| Comparative Example 1 | Structural formula (6)  | 30                                                           | 94                                        | 6                                         | 0.28                                   | 37                      | 0.37                                   | 89                      | E                                                                   |
| Comparative Example 2 | Structural formula (7)  | 29                                                           | 100                                       | 0                                         | 0.29                                   | 32                      | 0.41                                   | 106                     | E                                                                   |
| Comparative Example 3 | Structural formula (8)  | 18                                                           | 75                                        | 25                                        | Unable to measure sensitivity          | —                       | —                                      | —                       | —                                                                   |
| Comparative Example 4 | Structural formula (9)  | 18                                                           | 100                                       | 0                                         | Unable to measure sensitivity          | —                       | —                                      | —                       | —                                                                   |
| Comparative Example 5 | Structural formula (10) | —                                                            | 43                                        | 57                                        | 0.63                                   | 104                     | Unable to measure sensitivity          | —                       | —                                                                   |
| Comparative Example 6 | Structural formula (11) | 36                                                           | 52                                        | 48                                        | 0.52                                   | 90                      | 0.66                                   | 143                     | D                                                                   |
| Comparative Example 7 | Structural formula (12) | 40                                                           | 93                                        | 7                                         | 0.66                                   | 205                     | Unable to measure sensitivity          | —                       | —                                                                   |
| Comparative Example 8 | Structural formula (13) | 34                                                           | 95                                        | 5                                         | Unable to measure sensitivity          | —                       | —                                      | —                       | —                                                                   |

The foregoing results show that when a molecule of a hole transporting substance is formed of a compound consisting of a carbon atom and a hydrogen atom, or consisting of a carbon atom, a hydrogen atom, and an oxygen atom, an image defect such as image deletion under high-temperature and high-humidity conditions is efficiently suppressed. Further, an electrophotographic photosensitive member using a hole transporting substance free of any oxygen atom was more excellent.

In the results of the measurement of the sensitivity and the residual potential, Examples 1, 2, 3, 6, 8, 11, and 15 showed relatively good results. This is probably because the number of sp<sup>2</sup> carbon atoms involved in conjugation was relatively large, and the ratios of the number of sp<sup>2</sup> carbon atoms and sp<sup>3</sup> carbon atoms were suitable.

In the same mixed surface layer of a hole transporting substance and an amine-based hole transporting substance as that of Example 1, a good result is obtained when the hole transporting substance of the present invention is incorporated at about 80 mass %.

### Example 23

The aluminum cylinder used in Example 1 was used as a support. Next, 60 parts of barium sulfate particles covered with tin oxide (trade name: Passtran PC1, manufactured by MITSUI MINING & SMELTING CO., LTD.), 15 parts of titanium oxide particles (trade name: TITANIX JR, manufactured by TAYCA), 43 parts of a resole-type phenol resin (trade name: PHENOLITE J-325, manufactured by DIC Corporation, solid content: 70%), 0.015 part of silicone oil (trade name: SH28PA, manufactured by Dow Corning Toray Co., Ltd.), and 3.6 parts of silicone resin particles (trade name: TOSPEARL 120, manufactured by Momentive Performance Materials Inc.) were mixed in a mixed solvent of 50 parts of

2-methoxy-1-propanol and 50 parts of methanol, and the mixture was dispersed with a ball mill for about 20 hours to prepare a conductive-layer coating solution. The conductive-layer coating solution was applied onto the support by dipping, and the resultant coat was cured by heating for 1 hour at 140°C. to form a conductive layer having a thickness of 15 μm.

Next, 10 parts of a copolymerized nylon resin (trade name: AMILAN CM8000, manufactured by TORAY INDUSTRIES, INC.) and 30 parts of a methoxymethylated 6-nylon resin (trade name: TORESIN EF-30T, manufactured by Nagase ChemteX Corporation) were dissolved in a mixed solvent of 400 parts of methanol and 200 parts of n-butanol to prepare an undercoat-layer coating solution. The undercoat-layer coating solution was applied onto the conductive layer by dipping, and the resultant coat was dried by heating at a temperature of 100°C. for 30 minutes to form an undercoat layer having a thickness of 0.45 μm.

Next, the same charge generating layer as that of Example 1 was formed on the undercoat layer.

Next, 70 parts of the hole transporting substance represented by Exemplified Compound No. 56 and 100 parts of a polycarbonate resin (Iupilon 2800 manufactured by Mitsubishi Engineering-Plastics Corporation) were dissolved in 1,240 parts of monochlorobenzene to prepare a hole-transferring-layer coating solution. The hole-transferring-layer coating solution was applied onto the charge generating layer by dipping to form a coat, and the resultant coat was dried by heating at a temperature of 100°C. for 60 minutes to form a hole transporting layer (surface layer) having a thickness of 7 μm.

(Evaluation of Electrophotographic Photosensitive Member)

The same photosensitive member testing apparatus as that of Example 1 was used in the evaluation of the electrophoto-

## 115

graphic photosensitive member for its initial sensitivity and residual potential. First, a condition for a charging device was set so that the dark-area potential (Vd) of the electrophotographic photosensitive member became -600 (V) under a 23° C./50% RH environment. The photosensitive member was irradiated with monochromatic light having a wavelength of 780 nm, and the quantity of the light needed for reducing the potential of -600 (V) to -200 (V) was measured and defined as a sensitivity  $\Delta 400$  ( $\mu$ J/cm<sup>2</sup>). Further, the potential of the electrophotographic photosensitive member when the photosensitive member was irradiated with light having a quantity of 40 ( $\mu$ J/cm<sup>2</sup>) was measured as a residual potential V<sub>r</sub> (-V).

The electrophotographic photosensitive member was mounted onto the cyan station of a reconstructed machine of an electrophotographic copying machine (trade name: iR-ADV C5051) manufactured by Canon Inc. as an image evaluating apparatus, and was evaluated as described below.

First, a condition for a charging device was set so that the dark-area potential (Vd) of the electrophotographic photosensitive member became -600 (V) under a 23° C./50% RH environment. The photosensitive member was irradiated with laser light having a wavelength of 780 nm, the quantity of the light needed for reducing the potential of -600 (V) to -200 (V) was determined, and repeated image formation was performed by continuously outputting an evaluation chart, which was an A4 horizontal 5% image, on 1,000 sheets. The image formation was performed by setting the total quantity of a discharge current in the charging step to 350 ( $\mu$ A).

After the completion of the repeated image formation, the electrophotographic photosensitive member taken out of the image evaluating apparatus was immediately mounted onto the same photosensitive member testing apparatus as that described above, its sensitivity and residual potential were measured, and a variation between potentials before and after the repeated image formation was evaluated.

Next, an electrophotographic apparatus reconstructed so as to be capable of, for example, regulation and measurement so that the total current, and the DC component and AC component of a voltage to be applied to the charging roller could each be controlled was prepared as an electrophotographic apparatus. In addition, evaluation was performed while the power source of a heater accompanying the main body of the electrophotographic apparatus was turned off.

A cyan cartridge to be used in the electrophotographic apparatus was prepared, and the electrophotographic apparatus, the cartridge, and the electrophotographic photosensitive member were left to stand under a 30° C./80% RH environment for 24 hours or more. After that, the electrophotographic photosensitive member was mounted onto the cyan cartridge for image formation and evaluation. Then, an entire exposure image having a cyan color alone was output on A4 size plain paper and an image exposure light quantity was set so that a density on the paper measured with a spectral densitometer (trade name: X-Rite 504, manufactured by X-Rite Inc.) became 1.45.

Evaluation for image reproducibility was performed by setting the total quantity of a discharge current in the step of charging the electrophotographic photosensitive member to 350 ( $\mu$ A). A 1,000-sheet repeated image formation test was performed with a test chart having an image density ratio of 5% in this setting. After the completion of the repeated image formation, the electrophotographic photosensitive member was taken out of the electrophotographic apparatus together with the cartridge, and was left to stand under the same 30° C./80% RH environment in a dark place for 24 hours.

After that, the cartridge including the electrophotographic photosensitive member was mounted onto the same electro-

## 116

photographic apparatus again, an A4 horizontal 1-dot/1-space image having an output resolution of 600 dpi was formed, and the same evaluation as that of Example 1 was performed.

Table 2 shows the result of the evaluation for the electric potential variation due to repeated image formation, and the results of the evaluation for image characteristics under a high-temperature and high-humidity environment.

## Examples 24 to 40

Electrophotographic photosensitive members were each produced and evaluated in the same manner as in Example 23 except that the hole transporting substance used in the hole transporting layer of Example 23 was changed to a hole transporting substance shown in Table 2. Table 2 shows the results of the evaluation.

## Example 41

The hole transporting substance of Example 23 was changed as follows: 63 parts of the hole transporting substance represented by Exemplified Compound No. 56 and 7 parts of the hole transporting substance represented by the formula (5) were used as a mixture. Further, 100 parts of the same polycarbonate resin as that of Example 23 were dissolved in 1,240 parts of monochlorobenzene to prepare a hole-transferring-layer coating solution. An electrophotographic photosensitive member was produced in the same manner as in Example 23 except the foregoing. Further, the electrophotographic photosensitive member was evaluated in the same manner as in Example 23. Table 2 shows the results of the evaluation.

## Example 42

The hole transporting substance of Example 23 was changed as follows: 56 parts of the hole transporting substance represented by Exemplified Compound No. 56 and 14 parts of the hole transporting substance represented by the formula (5) were used as a mixture. Further, 100 parts of the same polycarbonate resin as that of Example 23 were dissolved in 1,240 parts of monochlorobenzene to prepare a hole-transferring-layer coating solution. An electrophotographic photosensitive member was produced in the same manner as in Example 23 except the foregoing. Further, the electrophotographic photosensitive member was evaluated in the same manner as in Example 23. Table 2 shows the results of the evaluation.

## Example 43

The hole transporting substance of Example 23 was changed as follows: 35 parts of the hole transporting substance represented by Exemplified Compound No. 56 and 35 parts of the hole transporting substance represented by the formula (5) were used as a mixture. Further, 100 parts of the same polycarbonate resin as that of Example 23 were dissolved in 1,240 parts of monochlorobenzene to prepare a hole-transferring-layer coating solution. An electrophotographic photosensitive member was produced in the same manner as in Example 23 except the foregoing. Further, the electrophotographic photosensitive member was evaluated in the same manner as in Example 23. Table 2 shows the results of the evaluation.

## Comparative Example 9

An electrophotographic photosensitive member was produced in the same manner as in Example 23 except that the

hole transporting substance of Example 23 was changed to the hole transporting substance represented by the formula (6), and the electrophotographic photosensitive member was similarly evaluated. Table 2 shows the results of the evaluation.

## Comparative Example 10

An electrophotographic photosensitive member was produced in the same manner as in Example 23 except that the hole transporting substance of Example 23 was changed to the hole transporting substance represented by the formula (7), and the electrophotographic photosensitive member was similarly evaluated. Table 2 shows the results of the evaluation.

## Comparative Example 11

An electrophotographic photosensitive member was produced in the same manner as in Example 23 except that the hole transporting substance of Example 23 was changed to the aromatic compound represented by the formula (8), and the electrophotographic photosensitive member was similarly evaluated. Table 2 shows the results of the evaluation.

## Comparative Example 12

An electrophotographic photosensitive member was produced in the same manner as in Example 23 except that the hole transporting substance of Example 23 was changed to the aromatic compound represented by the formula (9), and the electrophotographic photosensitive member was similarly evaluated. Table 2 shows the results of the evaluation.

## Comparative Example 13

An electrophotographic photosensitive member was produced in the same manner as in Example 23 except that the hole transporting substance of Example 23 was changed to the polyfluorene compound represented by the formula (10), and the electrophotographic photosensitive member was similarly evaluated. Table 2 shows the results of the evaluation.

## Comparative Example 14

An electrophotographic photosensitive member was produced in the same manner as in Example 23 except that the hole transporting substance of Example 23 was changed to the aromatic compound represented by the formula (11), and the electrophotographic photosensitive member was similarly evaluated. Table 2 shows the results of the evaluation.

## Comparative Example 15

An electrophotographic photosensitive member was produced in the same manner as in Example 23 except that the hole transporting substance of Example 23 was changed to the compound represented by the formula (12), and the electrophotographic photosensitive member was similarly evaluated. Table 2 shows the results of the evaluation.

## Comparative Example 16

An electrophotographic photosensitive member was produced in the same manner as in Example 23 except that the hole transporting substance of Example 23 was changed to the aromatic compound represented by the formula (13), and the electrophotographic photosensitive member was similarly evaluated. Table 2 shows the results of the evaluation.

TABLE 2

| No.                    | Kind of compound         | Hole transporting substance                                  |                                           |                                           | Initial potential at 23° C./50% RH     |                         |                                        |                                    | Potential after 1,000-sheet |     | endurance under high temperature and high humidity Image evaluation |  |  |
|------------------------|--------------------------|--------------------------------------------------------------|-------------------------------------------|-------------------------------------------|----------------------------------------|-------------------------|----------------------------------------|------------------------------------|-----------------------------|-----|---------------------------------------------------------------------|--|--|
|                        |                          | Number of sp <sup>2</sup> carbon atoms that form conjugation | Ratio of sp <sup>2</sup> carbon atoms (%) | Ratio of sp <sup>3</sup> carbon atoms (%) | Sensitivity Δ400 (μJ/cm <sup>2</sup> ) | Residual potential (-V) | Sensitivity Δ400 (μJ/cm <sup>2</sup> ) | Residual potential (-V)            |                             |     |                                                                     |  |  |
|                        |                          |                                                              |                                           |                                           |                                        |                         |                                        | Initial potential at 23° C./50% RH | endurance at 23° C./50% RH  |     |                                                                     |  |  |
| Example 23             | Exemplified Compound 56  | 44                                                           | 80                                        | 20                                        | 0.65                                   | 63                      | 0.65                                   | 66                                 | 0.65                        | 66  | A                                                                   |  |  |
| Example 24             | Exemplified Compound 17  | 28                                                           | 72                                        | 28                                        | 0.74                                   | 67                      | 0.76                                   | 70                                 | 0.76                        | 70  | A                                                                   |  |  |
| Example 25             | Exemplified Compound 24  | 28                                                           | 76                                        | 24                                        | 0.77                                   | 84                      | 0.78                                   | 89                                 | 0.78                        | 89  | A                                                                   |  |  |
| Example 26             | Exemplified Compound 42  | 36                                                           | 61                                        | 39                                        | 0.82                                   | 83                      | 0.82                                   | 97                                 | 0.82                        | 97  | B                                                                   |  |  |
| Example 27             | Exemplified Compound 58  | 44                                                           | 75                                        | 25                                        | 0.65                                   | 64                      | 0.67                                   | 69                                 | 0.67                        | 69  | A                                                                   |  |  |
| Example 28             | Exemplified Compound 63  | 40                                                           | 80                                        | 20                                        | 0.66                                   | 62                      | 0.66                                   | 64                                 | 0.66                        | 64  | A                                                                   |  |  |
| Example 29             | Exemplified Compound 64  | 40                                                           | 74                                        | 26                                        | 0.69                                   | 68                      | 0.71                                   | 77                                 | 0.71                        | 77  | A                                                                   |  |  |
| Example 30             | Exemplified Compound 67  | 40                                                           | 69                                        | 31                                        | 0.73                                   | 75                      | 0.75                                   | 83                                 | 0.75                        | 83  | A                                                                   |  |  |
| Example 31             | Exemplified Compound 72  | 40                                                           | 74                                        | 26                                        | 0.68                                   | 69                      | 0.70                                   | 74                                 | 0.70                        | 74  | A                                                                   |  |  |
| Example 32             | Exemplified Compound 85  | 38                                                           | 76                                        | 24                                        | 0.66                                   | 60                      | 0.68                                   | 64                                 | 0.68                        | 64  | A                                                                   |  |  |
| Example 33             | Exemplified Compound 92  | 44                                                           | 83                                        | 17                                        | 0.69                                   | 82                      | 0.70                                   | 88                                 | 0.70                        | 88  | A                                                                   |  |  |
| Example 34             | Exemplified Compound 115 | 48                                                           | 63                                        | 37                                        | 0.77                                   | 71                      | 0.80                                   | 81                                 | 0.80                        | 81  | B                                                                   |  |  |
| Example 35             | Exemplified Compound 119 | 44                                                           | 76                                        | 24                                        | 0.73                                   | 72                      | 0.74                                   | 77                                 | 0.74                        | 77  | A                                                                   |  |  |
| Example 36             | Exemplified Compound 127 | 68                                                           | 73                                        | 27                                        | 0.66                                   | 64                      | 0.68                                   | 70                                 | 0.68                        | 70  | A                                                                   |  |  |
| Example 37             | Exemplified Compound 176 | 40                                                           | 85                                        | 15                                        | 0.70                                   | 66                      | 0.72                                   | 69                                 | 0.72                        | 69  | B                                                                   |  |  |
| Example 38             | Exemplified Compound 180 | 40                                                           | 82                                        | 18                                        | 0.71                                   | 62                      | 0.72                                   | 65                                 | 0.72                        | 65  | A                                                                   |  |  |
| Example 39             | Exemplified Compound 191 | 40                                                           | 77                                        | 23                                        | 0.73                                   | 66                      | 0.75                                   | 68                                 | 0.75                        | 68  | B                                                                   |  |  |
| Example 40             | Exemplified Compound 210 | 44                                                           | 77                                        | 23                                        | 0.70                                   | 65                      | 0.71                                   | 68                                 | 0.71                        | 68  | B                                                                   |  |  |
| Example 41             | Exemplified Compound 56  | 44                                                           | 80                                        | 20                                        | 0.65                                   | 66                      | 0.66                                   | 78                                 | 0.66                        | 78  | B                                                                   |  |  |
| Example 42             | Exemplified Compound 56  | 44                                                           | 80                                        | 20                                        | 0.67                                   | 74                      | 0.70                                   | 79                                 | 0.70                        | 79  | B                                                                   |  |  |
| Example 43             | Exemplified Compound 56  | 44                                                           | 80                                        | 20                                        | 0.82                                   | 82                      | 0.83                                   | 96                                 | 0.83                        | 96  | C                                                                   |  |  |
| Comparative Example 9  | Structural formula (6)   | 30                                                           | 94                                        | 6                                         | 0.65                                   | 16                      | 0.70                                   | 87                                 | 0.70                        | 87  | E                                                                   |  |  |
| Comparative Example 10 | Structural formula (7)   | 29                                                           | 100                                       | 0                                         | 0.67                                   | 12                      | 0.81                                   | 131                                | 0.81                        | 131 | E                                                                   |  |  |

TABLE 2-continued

| No.                    | Kind of compound        | Hole transporting substance                                  |                                           |                                           | Initial potential at 23° C./50% RH     |                         | Potential after 1,000-sheet            |                         | endurance under high temperature and high humidity and high humidity Image evaluation |
|------------------------|-------------------------|--------------------------------------------------------------|-------------------------------------------|-------------------------------------------|----------------------------------------|-------------------------|----------------------------------------|-------------------------|---------------------------------------------------------------------------------------|
|                        |                         | Number of sp <sup>2</sup> carbon atoms that form conjugation | Ratio of sp <sup>2</sup> carbon atoms (%) | Ratio of sp <sup>3</sup> carbon atoms (%) | Sensitivity Δ400 (μJ/cm <sup>2</sup> ) | Residual potential (-V) | Sensitivity Δ400 (μJ/cm <sup>2</sup> ) | Residual potential (-V) |                                                                                       |
|                        |                         | atoms that form conjugation                                  | carbon atoms (%)                          | carbon atoms (%)                          | Δ400 (μJ/cm <sup>2</sup> )             | (-V)                    | Δ400 (μJ/cm <sup>2</sup> )             | (-V)                    |                                                                                       |
| Comparative Example 11 | Structural formula (8)  | 18                                                           | 75                                        | 25                                        | Unable to measure sensitivity          | —                       | —                                      | —                       | —                                                                                     |
| Comparative Example 12 | Structural formula (9)  | 18                                                           | 100                                       | 0                                         | Unable to measure sensitivity          | —                       | —                                      | —                       | —                                                                                     |
| Comparative Example 13 | Structural formula (10) | —                                                            | 43                                        | 57                                        | Unable to measure sensitivity          | —                       | —                                      | —                       | —                                                                                     |
| Comparative Example 14 | Structural formula (11) | 36                                                           | 52                                        | 48                                        | Unable to measure sensitivity          | —                       | —                                      | —                       | —                                                                                     |
| Comparative Example 15 | Structural formula (12) | 40                                                           | 93                                        | 7                                         | Unable to measure sensitivity          | —                       | —                                      | —                       | —                                                                                     |
| Comparative Example 16 | Structural formula (13) | 34                                                           | 95                                        | 5                                         | Unable to measure sensitivity          | —                       | —                                      | —                       | —                                                                                     |

The foregoing results show that when a hole transporting substance to be used in a surface layer (hole transporting layer) consists of a carbon atom and a hydrogen atom, or consists of a carbon atom, a hydrogen atom, and an oxygen atom, image deletion under high-temperature and high-humidity conditions is efficiently suppressed. Further, the use of a hole transporting substance consisting of a carbon atom and a hydrogen atom was more excellent.

In the results of the measurement of the sensitivity and the residual potential, Examples 23, 24, 32, 37, and 38 showed good results. This is probably because the number of sp<sup>2</sup> carbon atoms involved in conjugation was large, and the

Example 23 to form an undercoat layer having a thickness of 0.45 μm.

Next, 4.6 parts of a bisazo pigment represented by the following formula (14) as a charge generating substance and 2 parts of a butyral resin (butyralization degree: 68 mol %, weight-average molecular weight: 35,000) were mixed in 95 parts of cyclohexanone, and the mixture was dispersed with a sand mill for 36 hours to prepare a charge-generating-layer coating solution. The charge-generating-layer coating solution was applied onto the undercoat layer by dipping, and the resultant coat was dried by heating at a temperature of 80° C. for 15 minutes to form a charge generating layer having a thickness of 0.20 μm.



ratios of the number of sp<sup>2</sup> carbon atoms and sp<sup>3</sup> carbon atoms were suitable.

#### Example 44

The aluminum cylinder used in Example 1 was used as a support.

Next, the conductive-layer coating solution used in Example 23 was applied onto the support by dipping, and was cured in the same manner as in Example 23 to form a conductive layer having a thickness of 15 μm.

Next, the undercoat-layer coating solution used in Example 23 was applied onto the conductive layer by dipping, and was dried by heating in the same manner as in

Next, 80 parts of the hole transporting substance represented by Exemplified Compound No. 56 and 100 parts of a polycarbonate resin (Iupilon 2400) were dissolved in 600 parts of monochlorobenzene and 200 parts of tetrahydrofuran to prepare a hole-transporting-layer coating solution. The hole-transporting-layer coating solution was applied onto the charge generating layer by dipping, and the resultant coat was dried by heating at a temperature of 110° C. for 60 minutes to form a hole transporting layer having a thickness of 25 μm.

(Evaluation of Electrophotographic Photosensitive Member)

The electrophotographic photosensitive member of Example 44 was evaluated as described below.

## 121

A photosensitive member testing apparatus (CYN-THIA59) was used in the evaluation of the electrophotographic photosensitive member for its initial sensitivity and residual potential. First, a condition for a charging device was set so that the dark-area potential (Vd) of the electrophotographic photosensitive member became  $-700$  (V) under a  $23^\circ$  C./50% RH environment. The photosensitive member was irradiated with monochromatic light having a wavelength of  $530$  nm, and the quantity of the light needed for reducing the potential of  $-700$  (V) to  $-200$  (V) was measured and defined as a sensitivity  $\Delta 500$  ( $\mu\text{J}/\text{cm}^2$ ). Further, the potential of the electrophotographic photosensitive member when the photosensitive member was irradiated with light having a quantity of  $60$  ( $\mu\text{J}/\text{cm}^2$ ) was measured as a residual potential  $V_r$  (-V).

The electrophotographic photosensitive member was mounted onto the cyan station of a reconstructed machine of an electrophotographic copying machine (trade name: iR-ADV C5051) manufactured by Canon Inc. as an image evaluating apparatus, and was evaluated as described below.

First, a condition for a charging device was set so that the dark-area potential (Vd) of the electrophotographic photosensitive member became  $-700$  (V) under a  $23^\circ$  C./50% RH environment. Reconstruction was performed so as to allow the photosensitive member to be irradiated with laser light having a wavelength of  $530$  nm as a light source for image exposure. The photosensitive member was irradiated with laser light, and the quantity of the light needed for reducing

## 122

ment for 24 hours or more. After that, the electrophotographic photosensitive member was mounted onto the cyan cartridge for image formation and evaluation. Then, an entire exposure image having a cyan color alone was output on A4 size plain paper. After that, an image exposure light quantity was set so that a density on the output image measured with a spectral densitometer (trade name: X-Rite 504, manufactured by X-Rite Inc.) became 1.45.

Evaluation for image reproducibility was performed by 10 setting the total quantity of a discharge current in the step of charging the electrophotographic photosensitive member to  $300$  ( $\mu\text{A}$ ). A 1,000-sheet repeated image formation test was performed with a test chart having an image density ratio of 5% in this setting. After the completion of the repeated image 15 formation, the electrophotographic photosensitive member was taken out of the electrophotographic apparatus together with the cartridge, and was left to stand under the same  $30^\circ$  C./80% RH environment in a dark place for 24 hours.

After that, the cartridge was mounted onto the same electrophotographic apparatus again, an A4 horizontal 1-dot/1-space image having an output resolution of  $600$  dpi was formed, and the same evaluation as that of Example 1 was performed.

Table 3 shows the result of the evaluation for the electric 25 potential variation due to repeated image formation, and the results of the evaluation for image characteristics under a high-temperature and high-humidity environment.

TABLE 3

| No. | Kind of compound | Hole transporting substance                                |                                         |                                         | Initial potential at $23^\circ$ C./50% RH              |                         |                                                        | Potential after 1,000-sheet |      |    | endurance under high temperature and high humidity Image evaluation |
|-----|------------------|------------------------------------------------------------|-----------------------------------------|-----------------------------------------|--------------------------------------------------------|-------------------------|--------------------------------------------------------|-----------------------------|------|----|---------------------------------------------------------------------|
|     |                  | Number of $\text{sp}^2$ carbon atoms that form conjugation | Ratio of $\text{sp}^2$ carbon atoms (%) | Ratio of $\text{sp}^3$ carbon atoms (%) | Sensitivity $\Delta 500$ ( $\mu\text{J}/\text{cm}^2$ ) | Residual potential (-V) | Sensitivity $\Delta 500$ ( $\mu\text{J}/\text{cm}^2$ ) | Residual potential (-V)     |      |    |                                                                     |
|     |                  | Example 44                                                 | Exemplified Compound 56                 | 44                                      | 80                                                     | 20                      | 0.95                                                   | 40                          | 0.95 | 41 |                                                                     |
|     |                  |                                                            |                                         |                                         |                                                        |                         |                                                        |                             |      |    |                                                                     |

the potential of  $-700$  (V) to  $-200$  (V) was determined. After that, repeated image formation was performed by continuously outputting an evaluation chart, which was an A4 horizontal 5% image, on 1,000 sheets. The image formation was performed by setting the total quantity of a discharge current in the charging step to  $300$  ( $\mu\text{A}$ ).

After the completion of the repeated image formation, the electrophotographic photosensitive member taken out of the image evaluating apparatus was immediately mounted onto the same photosensitive member testing apparatus as that described above, its sensitivity and residual potential were measured, and a variation between potentials before and after the repeated image formation was evaluated.

Next, an electrophotographic apparatus reconstructed so as to be capable of, for example, regulation and measurement so that the total current, and the DC component and AC component of a voltage to be applied to the charging roller could each be controlled was prepared as an electrophotographic apparatus. In addition, evaluation was performed while the power source of a heater accompanying the main body of the electrophotographic apparatus was turned off.

A cyan cartridge to be used in the electrophotographic apparatus was prepared, and the electrophotographic apparatus, the cartridge, and the electrophotographic photosensitive member were left to stand under a  $30^\circ$  C./80% RH environ-

45 While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent 50 Applications No. 2013-045715, filed Mar. 7, 2013, and No. 2014-032962, filed Feb. 24, 2014 which are hereby incorporated by reference herein in their entirety.

What is claimed is:

1. An electrophotographic photosensitive member comprising:  
a support; and  
a photosensitive layer formed on the support,  
wherein the photosensitive layer comprises a charge generating layer and a surface layer, wherein,  
the charge generating layer contains at least one charge generating substance selected from the group consisting of hydroxygallium phthalocyanine, oxytitanium phthalocyanine, and chlorogallium phthalocyanine,  
the surface layer contains a hole transporting substance represented by the following formula (1)":

123



in the formula (1)'',  
 $R^1$  to  $R^6$ ,  $R^3$  to  $R^{6'}$ , and  $R^{3''}$  to  $R^{6''}$  each independently  
represents a hydrogen atom or an alkyl group,  
 $R^7$  represents a group derived from a pyrene,  
 $R^7'$  represents a group derived from a fluorene or an  
anthracene, and  
 $R^{7''}$  represents a group derived from a fluorene, a pyrene, an  
anthracene, a phenanthrene, or a fluoranthene,  
a ratio of a number of  $sp^3$  carbon atoms is 15% or more and  
35% or less based on a total number of carbon atoms in  
the hole transporting substance, and  
a thickness of the photosensitive layer is 5  $\mu m$  or more and  
10  $\mu m$  or less.

2. An electrophotographic apparatus comprising: the elec-  
trophotographic photosensitive member according to claim  
1; a charging device; an exposing device; a developing  
device; and a transferring device.

3. A process cartridge detachably mountable to a main  
body of an electrophotographic apparatus, wherein the pro-  
cess cartridge integrally supports: the electrophotographic  
photosensitive member according to claim 1; and at least one  
device selected from the group consisting of a charging  
device, a developing device, and a cleaning device.

4. The electrophotographic photosensitive member  
according to claim 1, wherein  
in the formula (1)'',  
 $R^1$  represents a tert-butyl group,  
 $R^2$  to  $R^6$ ,  $R^3$  to  $R^{6'}$ , and  $R^{3''}$  to  $R^{6''}$  each independently  
represents a hydrogen atom or an alkyl group,

20

25

30

15

124

$R^7$  represents a group derived from a pyrene,  
 $R^7'$  represents a group derived from a fluorene, and  
 $R^{7''}$  represents a group derived from a fluorene or a pyrene.

5. The electrophotographic photosensitive member  
according to claim 1, wherein the charge generating layer  
contains hydroxygallium phthalocyanine.

6. The electrophotographic photosensitive member  
according to claim 5, wherein the hydroxygallium phthalocy-  
anine is a hydroxygallium phthalocyanine crystal of a crys-  
tal form which has peaks at Bragg angles 20 in  $CuK\alpha$  char-  
acteristic X-ray diffraction of  $7.4^\circ \pm 0.3^\circ$  and  $28.2^\circ \pm 0.3^\circ$ .

7. The electrophotographic photosensitive member  
according to claim 1, wherein the thickness of the photosen-  
sitive layer is 5  $\mu m$  or more and 8  $\mu m$  or less.

8. The electrophotographic photosensitive member  
according to claim 1, wherein the hole transporting substance  
is represented by the following formula No. 56:

No. 56



\* \* \* \* \*